

# United States Patent [19]

Yoshida et al.

[11] Patent Number: 5,066,571

[45] Date of Patent: Nov. 19, 1991

[54] **METHOD FOR PROCESSING A SILVER HALIDE COLOR PHOTOSENSITIVE MATERIAL**

[75] Inventors: Kazuaki Yoshida; Takatoshi Ishikawa, both of Kanagawa, Japan

[73] Assignee: Fuji Photo Film Co., Ltd., Kanagawa, Japan

[21] Appl. No.: 416,690

[22] Filed: Oct. 3, 1989

[30] **Foreign Application Priority Data**

Oct. 3, 1988 [JP] Japan ..... 63-249250

[51] Int. Cl.<sup>5</sup> ..... G03C 5/24

[52] U.S. Cl. ..... 430/489; 430/268; 430/434; 430/484; 430/486; 430/490

[58] **Field of Search** ..... 430/268, 399, 486, 489, 430/490, 434, 447, 448, 484

[56] **References Cited**

**U.S. PATENT DOCUMENTS**

4,159,245 6/1979 Matsushita et al. ..... 430/399  
4,797,351 1/1989 Ishikawa et al. ..... 430/399  
4,897,339 1/1990 Andoh et al. ..... 430/484  
4,914,009 4/1990 Ueda et al. ..... 430/489  
4,933,265 6/1990 Inoue et al. ..... 430/489

**FOREIGN PATENT DOCUMENTS**

0312984 4/1989 European Pat. Off. .

1-05948 4/1989 Japan .  
1-16639 5/1989 Japan .

**OTHER PUBLICATIONS**

A Derwent Abstract of Japan No. A1-105948 is attached.

*Primary Examiner*—Hoa Van Le  
*Attorney, Agent, or Firm*—Sughrue, Mion, Zinn  
Macpeak & Seas

[57] **ABSTRACT**

A method for processing a silver halide color photosensitive material is disclosed.

The method comprises developing a color photographic light-sensitive material composed of a support having thereon at least one light-sensitive silver halide emulsion layer containing a silver halide comprising at least 98 mol % silver chloride;

in a color developer solution comprising a primary amine color developing agent, and having a chloride ion concentration of from  $4 \times 10^{-2}$  to  $1 \times 10^{-1}$  mol/l, and a bromide ion concentration of from  $5 \times 10^{-5}$  to  $5 \times 10^{-4}$  mol/l.

When used in rapid processing methods, the method according to the invention prevents fogging streaks, and provides high maximum density and low minimum density images.

**14 Claims, No Drawings**

## METHOD FOR PROCESSING A SILVER HALIDE COLOR PHOTOSENSITIVE MATERIAL

### FIELD OF THE INVENTION

The present invention relates to a method for processing silver halide color photographic photosensitive materials. More particularly, the invention relates to a development processing method which uses a high silver chloride photographic photosensitive material, providing excellent development characteristics and desilvering characteristics.

### BACKGROUND OF THE INVENTION

The trends to shorter delivery times for finished work and reduction of laboratory operations in photographic processing of color photographic photosensitive material in recent years have required processing time to be shortened. The usual methods of shortening the times required for different processing stages are to raise the temperature and to increase the amount of replenishment, and there have also been proposed many methods of stronger agitation and methods in which various types of accelerators are added.

To increase the speed of color development and/or reduce replenishment amounts, a method is known for processing color photographic photosensitive materials containing silver chloride emulsions instead of the silver bromide emulsions or silver iodide emulsions of popular conventional use. For example, PCT WO-87-04534 discloses a method for rapid processing of high silver chloride color photographic photosensitive material with a color development solution which contains essentially no sulfite or benzyl alcohol.

However, it has been found that streaky fogging occurs when development processing is performed by this method in an automatic paper development unit. It is surmized that this is "in-solution pressure sensitization streaking" in which streaky fogging occurs because the photosensitive material is bruised and pressure sensitized when it comes into contact with rollers in the development tank of an automatic development unit.

It has also been found that in continuous processing, fluctuation in photographic characteristics (especially the minimum density) occurs and there is considerable staining of the white background.

Thus, rapid development processing using high silver chloride color photographic photosensitive materials has the major problems of pressure sensitization fogging in the solution and fluctuation in photographic characteristics, and there is therefore a strong demand for resolution of these problems.

Use of the organic antifoggants disclosed in JP-A-58-95345 and JP-A-59-232342 (the term "JP-A" as used herein means an "unexamined published Japanese patent application") is known as a means for reducing fluctuation in photographic characteristics (and especially fogging) that occurs during continuous processing by rapid processing methods using high silver chloride color photographic photosensitive materials. However, these antifoggants have insufficient fogging prevention effects and fail to prevent pressure sensitization streaks in solutions, or the increase in the minimum density as continuous processing proceeds, and it has been found that when large amounts are used there is a decrease in the maximum density.

JP-A-61-70552 discloses a method for reducing the amount of development solution replenishment in

which use is made of high silver chloride color photographic photosensitive material and addition of replenishment solution is made in an amount such that there is no overflow to the development bath during development. JP-A-63-106655 teaches a method in which, in order to stabilize processing, a silver halide color photographic photosensitive material whose silver halide emulsion layers have a high silver chloride content is developed with a color development solution containing a chloride at higher than a set concentration and a hydroxylamine-based compound.

JP-A-63-106655 discloses a method of processing 70 mol % or more silver chloride photosensitive material using a development solution in which  $2 \times 10^{-2}$  moles or more of a chloride have been included.

With these methods, however, the above-described pressure sensitization streaks occur in processing by an automatic development unit, along with fluctuation in photographic characteristics during continuous processing, and these methods fail to resolve the problems noted above.

### SUMMARY OF THE INVENTION

A first object of the invention is to provide a rapid development processing method in which a high silver chloride color photographic photosensitive material is used, in which the occurrence of streaky fogging is prevented.

A second object of the invention is to provide a development processing method for a high silver chloride color photographic photosensitive material providing excellent photographic characteristics, i.e., the maximum density is high and the minimum density is low in rapid processing, and there is marked inhibition of fluctuation of photographic characteristics (especially the minimum density) during continuous processing.

It has now been found that these and other objects of the invention are achieved by a method for processing a silver halide color photosensitive material which comprises developing a color photographic lightsensitive material comprising a support having thereon at least one light-sensitive silver halide emulsion layer containing a silver halide comprising at least 80 mol % silver chloride;

in a color developer solution comprising a primary amine color developing agent, and having a chloride ion concentration of from  $3.5 \times 10^{-2}$  to  $1.5 \times 10^{-1}$  mol/l, and a bromide ion concentration of from  $3.0 \times 10^{-5}$  to  $1.0 \times 10^{-3}$  mol/l.

### DETAILED DESCRIPTION OF THE INVENTION

Chloride ions are well-known as an agent for preventing fogging but their effects are slight and even if they are used in large quantities they fail to completely prevent an increase in fogging during the course of continuous processing or streaky fogging that occurs in development by an automatic development unit, and they can even have the undesirable effect of slowing down development and lowering the maximum density.

Bromide ions too are well-known as an agent for preventing fogging. Although, depending on the amount added, they can prevent fogging during continuous processing and streaky pressure fogging, they are not suitable for practical use since they inhibit development and cause a lowering of the maximum density and sensitivity.

As the result of much investigation, the present inventors have discovered that if processing is performed using a high silver chloride photosensitive material with a silver chloride content of 80 mol % or more and a color development solution containing  $3.5 \times 10^{-2}$  to  $1.5 \times 10^{-1}$  mol/l of chloride ions and  $3.0 \times 10^{-5}$  to  $1.0 \times 10^{-3}$  mol/l of bromide ions, occurrence of streaky pressure fogging in processing by an automatic development unit and fluctuation in photographic characteristics (especially the minimum density) in the course of continuous processing are prevented without a loss of maximum density, and also the amount of residual silver is markedly reduced.

These effects are not observed with either bromide ions or chloride ions used alone, and it is unpredictable and surprising that they are achieved in combination within the concentrations of the invention.

Without being bound in any way by theory, it is considered likely that streaky pressure fogging which occurs in automatic development unit processing is the result of intensification and formation of fogging nuclei in portions that have been subjected to pressure when excessive pressure is imposed on photosensitive material in a color development solution following exposure. This fogging is different from fogging in the form of density resulting from development of unexposed portions.

It is considered likely that the inclusion of suitable amounts of bromide ions and chloride ions in the development solution in the invention effects selective inhibition of fogging nuclei, and thus inhibits fogging without slowing down development or reducing the maximum density or speed. This selective development inhibition effect that is caused by combinations of bromide ions and chloride ions cannot be explained simply in terms of a change in the silver ion reduction potential due to the presence of halogens and it is considered likely that the phenomenon is considerably affected by the way in which the bromide ions and chloride ions are adsorbed on silver halide grains.

The inhibition of fluctuation of photographic characteristics during continuous processing cannot be explained simply as inhibition of this fluctuation through a balance between high development activity brought about by use of a high silver chloride emulsion and a reduction in activity due to the presence of suitable amounts of bromide ions, i.e., through high activity-high inhibition type development.

With respect to the marked inhibition of desilvering faults, it is known that high silver chloride emulsions are liable to cause desilvering faults. The present inventors have discovered that the cause of desilvering faults is the formation of silver sulfite. It is considered that the presence of suitable amounts of bromide ions and chloride ions in the development solution changes the manner in which halogens are adsorbed on developed silver and thereby inhibits the formation of silver sulfite.

The invention will now be described in greater detail.

The silver halide emulsion is composed substantially of silver chloride. What is meant here by substantially, is that the silver chloride content relative to the total amount of silver halide is 80 mol % or more and preferably 95 mol % or more and still more preferably 98 mol % or more. For rapidity, the higher the silver chloride content the better.

For rapid development, desilvering characteristics and prevention of pressure sensitization streaks, it is preferred that the amount of coated silver in the silver

halide photosensitive material of the invention be not more than  $0.80 \text{ g/m}^2$ . This not only reduces the amount of silver but also reduces the film thickness. A coated silver quantity of  $0.75 \text{ g/m}^2$  or less is more preferred,  $0.65 \text{ g/m}^2$  or less being particularly preferred. The lower limit is suitably  $0.3 \text{ g/m}^2$ .

It is necessary that the color development solution have a chloride ion concentration of  $3.5 \times 10^{-2}$  to  $1.5 \times 10^{-1}$  mol/l and preferably the concentration is  $4 \times 10^{-2}$  to  $1.0 \times 10^{-1}$  mol/l. A chloride ion concentration of more than  $1.5 \times 10^{-1}$  mol/l has the drawback that it slows down development and fails to provide rapidity and a high maximum density. At less than  $3.5 \times 10^{-2}$  mol/l, it is not possible to prevent streaky pressure fogging, in addition to which there is considerable fluctuation in photographic characteristics (especially the minimum density) during the course of continuous processing and the amount of residual silver is large.

It is necessary that the color development solution have a bromide ion concentration of  $3.0 \times 10^{-5}$  to  $1.0 \times 10^{-3}$  mol/l and preferably the concentration is  $5.0 \times 10^{-5}$  to  $5 \times 10^{-4}$  mol/l. If the bromide ion concentration is more than  $1.0 \times 10^{-3}$  mol/l, development is slowed down and there is a loss of the maximum density and speed. If it is less than  $3.0 \times 10^{-5}$  mol/l, it is not possible to prevent streaky pressure fogging and it is not possible to prevent desilvering faults or fluctuation in photographic characteristics (especially the minimum density) as continuous processing proceeds.

The chloride ions and bromide ions may be added directly to the development solution or may be eluted from the photosensitive material into the development solution. A suitable measure for increasing the amount eluted from sensitive material is to reduce the amount of development solution replenishment.

Sodium chloride, potassium chloride, ammonium chloride, nickel chloride, magnesium chloride, manganese chloride, calcium chloride and cadmium chloride can be used as chloride ion donor substances when direct addition to the color development solution is made and sodium chloride and potassium chloride are preferred.

These may be supplied in the form of salts having counter ion of fluorescent brightness that are added to the development solution. Sodium bromide, potassium bromide, ammonium bromide, lithium bromide, calcium bromide, magnesium bromide, manganese bromide, nickel bromide, cadmium bromide, cerium bromide and thallium bromide may be used as bromide ion donor substances, and preferred are potassium bromide and sodium bromide.

In cases where the ions are eluted from the photosensitive material into the development solution, both the chloride ions and the bromide ions may be supplied from an emulsion or they may be supplied from a portion other than an emulsion.

From the point of view of processing stability during continuous processing and prevention of streaky pressure fogging, the color development solution in the invention preferably contains substantially no sulfite ions, this can be achieved by not using the development solution for a long time, so as to suppress deterioration of the development solution. Also, physical means such as use of a floating cover or reduction of the degree of opening of the development bath can be used, or controlling the development solution temperature or chemical means such as addition of organic preservatives in



In formula (II),  $R^{31}$ ,  $R^{32}$  and  $R^{33}$  are preferably hydrogen or  $C_{1-10}$  alkyl groups, and in most preferably  $R^{31}$  and  $R^{32}$  are hydrogen.

In formula (II),  $R^{34}$  is preferably an  $C_{1-10}$  alkyl,  $C_{6-10}$  aryl,  $C_{1-10}$  alkoxy,  $C_{1-10}$  carbamoyl or amino group, and an alkyl or substituted alkyl group is particularly preferred. Preferred alkyl group substituents include carboxyl, sulfo, nitro, amino and phosphono groups.  $X^{31}$  is preferably  $-CO-$  or  $-SO_2-$  is most preferably  $-CO-$ .

Specific examples of compounds of formula (II) are as follows, but the present invention is not to be construed as being limited thereto.



-continued



-continued



In the formula, X represents a trivalent atomic group needed for completing a condensed ring, and R<sup>1</sup> and R<sup>2</sup>, which may be the same or different, each represents alkylene, arylene, alkenylene or aralkylene groups.

Particularly preferred compounds represented by formula (IV) are compounds represented by formulae (IV-a) and (IV-b):

(IV-a)

III-7



5

In the formula, X<sup>1</sup> represents

III-8



10

III-9



15

III-10 R<sup>1</sup> and R<sup>2</sup> have the same definition as in formula (IV), and R<sup>3</sup> represents the same group as R<sup>1</sup> and R<sup>2</sup>, or is

III-11

III-12

20



III-13

The case where X<sup>1</sup> is

III-14

25



III-15

III-16 30 in general formula (IV-a) is preferred. The number of carbon atoms of each of R<sup>1</sup>, R<sup>2</sup> and R<sup>3</sup> is preferably 6 or less, and still more preferably 3 or less, the case and most preferably 2.III-17 35 R<sup>1</sup>, R<sup>2</sup> and R<sup>3</sup> are preferably alkylene or arylene groups and are most preferably alkylene groups.

(IV-b)

R<sup>1</sup>

III-18 40



III-19

45 In the formula, R<sup>1</sup> and R<sup>2</sup> have the same definition as in formula (IV).The number of carbon atoms of R<sup>1</sup> and R<sup>2</sup> is preferably 6 or less. R<sup>1</sup> and R<sup>2</sup> are preferably alkylene or arylene groups and are most preferably alkylene groups.

III-20

50 Among compounds represented by formulae (IV-a) and (IV-b), compounds represented by formula (IV-a) are particularly preferred.

55 Specific compounds represented by formulae (IV-a) and (IV-b) are as follows, but the present invention is (IV) not to be construed as being limited thereto.

IV-1



60



IV-2

65

-continued



IV-10      The above organic preservatives are available as commercial products, and they can be synthesized by the methods disclosed in Japanese Patent Applications 62-124038 and 62-24374.

IV-11      A more detailed description of the color development solutions that are employed in the invention is now provided.

IV-12      The color development solutions employed in the invention contain known primary aromatic amine developing agents. Preferred examples are p-phenylenediamines, typical examples of which follow, but the present invention is not to be construed as being limited thereto:

D-1 N,N-diethyl-p-phenylenediamine  
 D-2 4-[N-ethyl-N-( $\beta$ -hydroxyethyl)amino]aniline  
 D-3 2-methyl-4-[N-ethyl-N-( $\beta$ -hydroxyethyl)amino]aniline

D-4 4-amino-3-methyl-N-ethyl-N-( $\beta$ -methanesulfonamidoethyl)aniline

These p-phenylenediamine derivatives may also be salts such as sulfates, hydrochlorides or p-toluenesul-

fonates. These primary aromatic amine developing agents are used in concentrations that are preferably about 1 g to 20 g and still more preferably about 0.5 to about 10 g per 1 liter of development solution.

The pH of the color development solution used in this invention is preferably 9 to 12 and still more preferably 9 to 11.0. Other known development solution components may be included in the color development solution.

Preferably, various buffers are employed in order to maintain the above-described pH. Examples of buffers include sodium carbonate, potassium carbonate, sodium bicarbonate, potassium bicarbonate, trisodium phosphate, tripotassium phosphate, disodium phosphate, dipotassium phosphate, sodium borate, potassium borate, sodium tetraborate (borax), potassium tetraborate, sodium o-hydroxybenzoate (sodium salicylate), potassium o-hydroxybenzoate, sodium 5-sulfo-2-hydroxybenzoate (sodium 5-sulfosalicylate) and potassium 5-sulf-2-hydroxybenzoate (potassium 5-sulfosalicylate).

The amount of such buffers added to the color development solution is preferably 0.1 mol/l or more, 0.1 to 0.4 mol/l being particularly preferred.

In addition, various chelating agents may be used in the color development solution for preventing the precipitation of calcium and magnesium or in order to improve the solution's stability.

Specific examples of chelating agents are as follows, but the present invention is not to be construed as being limited thereto; Nitrilotriacetic acid, diethylenetriaminepentaacetic acid, ethylenediaminetetraacetic acid, triethylenetetraminehexaacetic acid, N,N,N-trimethylenephosphonic acid, ethylenediamine-N,N,N',N'-tetramethylene-phosphinic acid, 1,3-diamino-2-propanoltetraacetic acid, transcyclohexanediamine-tetraacetic acid, nitrilotripropionic acid, 1,2-diamino-propanetetraacetic acid, hydroxyethyliminodiacetic acid, glycol ether diaminetetraacetic acid, hydroxyethylene-diaminetetraacetic acid, ethylenediamine-ortho-hydroxyphenyl-acetic acid, 2-phosphonobutane-1,2,4-tricarboxylic acid, 1-hydroxyethylidene-1,1-diphosphonic acid, N,N'-bis(2-hydroxybenzyl)-ethylenediamine-N,N'-diacetic acid, catechol-3,4,6-trisulfonic acid, catechol-3,5-disulfonic acid, 5-sulfosalicylic acid, and 4-sulfosalicylic acid.

It is satisfactory if the amount of these chelating agents added is sufficient to sequester metal ions in the color development solution. For example, the amount is around 0.1 to 10 g per 1 liter.

If required, the thioether compounds noted in e.g., JP-B-37-16088, JP-B-37-5987, JP-B-38-7826, JP-B-44-12380 and JP-B-45-9019 and U.S. Pat. No. 3,813,247; the p-phenylenediamine compounds noted in JP-A-52-49829 and JP-A-50-15554; the quaternary ammonium salts noted in, e.g., JP-A-50-137726, JP-B-44-30074, JP-A-56-156826 and JP-A-52-43429; the p-amino-phenols disclosed in U.S. Pat. Nos. 2,610,122 and 4,119,462; the amine compounds disclosed in, e.g., U.S. Pat. Nos. 2,494,903, 3,128,182, 4,230,796 and 3,253,919, JP-B-41-11431 and U.S. Pat. Nos. 2,482,546, 2,596,926 and 3,582,346; or the polyalkylene oxides noted in, e.g., JP-B-37-16088, JP-B-42-25201, U.S. Pat. No. 3,238,183, JP-B-41-11431, JP-B-42-23883 and U.S. Pat. No. 3,532,501, may be added as development accelerators and as well as these substances 1-phenyl-3-pyrazolidones, hydrazines, mesoionic compounds, ionic compounds and imidazoles may be added as required.

Preferably, the color development solution is substantially free of benzyl alcohol. Substantially free as used herein means a content of not more than 2.0 ml per 1 liter of color development solution and preferably none at all. If the solution is essentially free of benzyl alcohol there is less fluctuation of photographic characteristics in continuous processing and better results are achieved.

In the invention, chloride ions and bromine ions may be added and any antifogging may be added as required. Alkali metal compounds such as potassium iodide and organic antifogging agents may be used as antifogging agents. Benzotriazole, 6-nitrobenzimidazole, 5-nitroisoindazole, antifogging agents may be used as antifogging agents. 5-methylbenzotriazole, 5-nitrobenzotriazole, 5-chlorobenzotriazole, 2-thiazolylbenzimidazole, 2-thiazolylmethylbenzimidazole, indazole, hydroxyazaindolidine, adenine and similar nitrogen-containing heterocyclic compounds are representative examples of organic antifogging agents.

Preferably, a brightening agent is included in the color development solution that is used in the invention. 4,4'-Diamino-2,2'-disulfostibene compounds are preferred as brightening agents. The amount added is 0 to 10 g/l and preferably 0.1 to 6 g/l.

The processing temperature of the color development solution of the invention is 20° to 50° C. and preferably 30° to 40° C. and the development processing time is 20 seconds to 5 minutes and preferably 30 seconds to 2 minutes.

Normally in color development the development solution is replenished.

The amount of replenishment depends on the photosensitive material being processed and generally it is on the order of 180 to 1000 ml per 1 square meter of photosensitive material. Replenishment is a means of keeping the color development solution composition constant so as to avoid changes in the characteristics of the development finish due to changes in composition concentrations in development processing in which a large amount of photosensitive material is continuously processed with an automatic development machine. From the point of view of cost and environmental pollution it is preferred to keep the amount of replenishment small, since replenishment inevitably gives rise to produce large amount of overflow solution. The preferred replenishment quantity is 20 to 150 ml per 1 m<sup>2</sup> of photosensitive material. Although there are some differences depending on the photosensitive material, a replenishment quantity of 20 ml per 1 m<sup>2</sup> of photosensitive material is approximately equal to the amount of processing solution carried out by the photosensitive material, and so overflow is essentially eliminated with this quantity. The present invention is useful in low-replenishment of this kind.

In the invention, desilvering is effected after color development. The desilvering stage generally consists of a bleaching step and a fixing step but the simultaneous performance of these steps is particularly preferred.

The bleaching solution or bleach-fix solution used in the invention may contain rehalogenation agents such as bromides (e.g., potassium bromide, sodium bromide, ammonium bromide), chlorides (e.g., potassium chloride, sodium chloride, ammonium chloride) or iodides (e.g., ammonium iodide). If required, one or more inorganic or organic acids which possess pH buffering capacity or alkali metal or ammonium salts thereof such as

boric acid, borax, sodium metaborate, acetic acid, sodium acetate, sodium carbonate, potassium carbonate, phosphorous acid, phosphoric acid, sodium phosphate, citric acid, sodium citrate or tartaric acid, and corrosion preventives such as ammonium nitrate and guanidine may be added.

The fixer used in the bleach-fix or fixing solution in the invention may be a known fixer, i.e., a thiosulfate such as sodium thiosulfate or ammonium thiosulfate; a thiocyanate such as sodium thiocyanate or ammonium thiocyanate; a thioether compound such as ethylenebis-thioglycolic acid or 3,6-dithia-1,8-octanediol or a thiourea or similar water-soluble silver halide solvent, used alone or as a mixture of two or more substances. It is also possible to use, e.g., the special bleach-fixing solution disclosed in JP-A-55-155354 consisting of a fixer and a large amount of a halide such as potassium iodide. In the invention, use of a thiosulfate, especially ammonium thiosulfate, is preferred. The amount of fixer per 1 liter is preferably 0.3 to 2 moles and more preferably is in the range 0.5 to 1.0 moles.

The pH of the bleach-fix solution or bleaching solution in the invention is preferably 3 to 10 and more preferably 5 to 9. A pH lower than this improves desilvering but promotes deterioration of the solution and achromatization of cyan dyes. If the pH is higher than this region desilvering is slowed down and stains are liable to be produced.

If required, substances such as hydrochloric acid, sulfuric acid, nitric acid, acetic acid, bicarbonates, ammonia, caustic potash, caustic soda, sodium carbonate and potassium carbonate may be added in order to regulate the pH.

The bleach-fix solution may also contain various brightening agents, antifoaming agents, surfactants, or organic solvents such as polyvinylpyrrolidone and methanol.

The bleach-fix solution or fixing solution in the invention contains a preservative in the form of a sulfite (e.g., sodium sulfite, potassium sulfite, ammonium sulfite), a bisulfite (e.g., ammonium bisulfite, sodium bisulfite, potassium bisulfite), a metabisulfite (e.g., potassium metabisulfite, sodium metabisulfite, ammonium metabisulfite) or similar sulfite-ion releasing compound. Converted to sulfite ions, the amount of such compounds included is preferably 0.02 to 0.50 mol/l and more preferably 0.04 to 0.40 mol/l.

It is normal practice to add sulfites as preservatives, but it is also possible to add ascorbic acid, carbonyl bisulfite adducts, sulfinic acids or carbonyl compounds.

Substances such as buffers, brightening agents, chelating agents and antifungal agents may be used if required.

Generally, the silver halide color photographic photosensitive material of the invention is subjected to a washing and/or stabilization stage after fixing, bleach-fixing and similar desilvering treatment.

The amount of washing water in the washing stage can be set in accordance with a wide range of conditions such as the characteristics of the photosensitive material (which, depend on the material used for the couplers), the purpose of the material, the washing water temperature, the number of washing tanks (the number of stages) and whether a counterflow or direct flow replenishment system is used. The relation between the amount of water and the number of washing stages in a multistage counterflow system can be determined by the method described in the *Journal of the*

*Society of Motion Picture and Television Engineers, Vol. 64, p. 248-253 (May 1955).*

The multistage counterflow system there described makes it possible to greatly reduce the amount of washing water, but creates problems such as the proliferation of bacteria and adhesion to the photosensitive material of suspended matter that forms because of the increased dwell-time of water in the tanks. A very effective measure that may be employed to resolve such problems in processing of the color photosensitive material of the invention is to use the method disclosed in JP-A-61-131632 for reducing calcium and magnesium. Alternatively, isothiazolone compounds or thiabenzazoles disclosed in JP-A-57-8542, sodium chloroisocyanurate or similar chlorine-based bactericides, benzotriazoles or the bactericides described by Dr. Horiguchi in *Sakkin-Bobaizai no Kaqaku (Chemistry of Antibacterial-Antifungal Agents)*, *Biseibutsu no Mekkin, Sakkin, Bobai Gijutsu (Microorganism Sterilization, Bactericidal Antifungal Technology)* edited by the Eisei Gijutsukai (Hygiene Technology Institute) or *Bokin-Bobai Jiten (Dictionary of Bacteria - Fungus Prevention)* edited by the Nihon Bokin Bobai Gakkai (Japan Antibacterial Antifungal Institute) can be used.

The pH of the washing water during processing of the photosensitive material of the invention is 4 to 9 and preferably 5 to 8. The washing water temperature and the washing time can be widely varied depending on the photosensitive material's characteristics and intended use, but generally values in the range of 20 seconds to 5 minutes at 25° to 40° C., are selected.

The photosensitive material of the invention can also be processed directly by a stabilization solution without being washed. Any of the known methods disclosed in, e.g., JP-A-57-8543, JP-A-58-14834, JP-A-59-184343, JP-A-60-220345, JP-A-60-238832, JP-A-60-239784, JP-A-60-239749, JP-A-61-4054 and JP-A-61-118749 may be used for this form of stabilization treatment. In particular, a stabilization bath containing compounds such as 1-hydroxyethylidene-1,1-diphosphonic acid, 5-chloro-2-methyl-4-isothiazolin-3-one, bismuth compounds and ammonium compounds, is preferably used.

In some cases, stabilization treatment is effected after washing treatment, by using a stabilization bath which contains formalin and a surfactant, as the last bath for the photographic color photosensitive material.

The processing stages time in the invention is defined as the time from when the photosensitive material comes into contact with the color development solution unit it exists from the final bath (usually a washing or stabilization bath) and the advantages of the invention are particularly marked when this rapid treating process stages time is 4 minutes 30 seconds or less or better 4 minutes or less.

The rapid treating process according to the present invention generally comprises following steps:

(A) Developing - Bleaching - Fixing - Washing - (Stabilizing)

(B) Developing - Bleach-fixing - Washing - (Stabilizing)

(C) Developing - Bleaching - Bleach-fixing - Washing - (Stabilizing)

In the above steps Stabilizing step is optional.

The silver halide color photographic photosensitive material of the invention is now described in greater detail.

The silver halide emulsion of the invention is composed substantially of silver chloride. What is meant

here by 'substantially' is that the silver chloride content relative to the total amount of silver halide is 80 mol % or more and preferably 95 mol % or more and still more preferably 98 mol % or more. From the point of view of rapidity, the higher the silver chloride content the better. A small amount of silver bromide or silver iodide may be included in the high silver chloride of the invention. This offers many advantages for photosensitivity, by increasing the amount of light absorbed, strengthening the adsorption of spectrally sensitized dyes or weakening the effects of desensitization due to spectrally sensitized dyes.

The silver halide included in the silver halide emulsion of the photographic photosensitive material that is used in the invention may have different phases in internal and outer layers or may have a multiphase structure in a bonded arrangement, or the grains may have a uniform phase throughout. The grain may be a mixture of these types.

The silver halide grains in the photographic emulsion may be cubic, octahedral, tetradecahedral or similar regular crystals, or may have a spheroidal, tabular-shaped or similar irregular crystal shapes or crystal defects, such as twin crystal planes, or they may have combinations of these forms.

The silver halide grains may be microscopic grains with a grain diameter of about 0.2 microns or less or large-size grains with a projected area diameter of up to about 10 microns, and the emulsion may be a polydisperse emulsion or a monodisperse emulsion.

A silver halide photographic emulsion used in the invention can be prepared by methods described in *Research Disclosure* (RD) No. 17643 (December 1978), pages 22-23, I. Emulsion Preparation and Types.

Monodisperse emulsions such as those disclosed in e.g., U.S. Pat. Nos. 3,574,628 and 3,655,394 and U.K. Patent 1,413,748 are suitable.

It is also possible to use tabular grains with an aspect ratio of about 5 or more in the invention. Tabular grains can be simply prepared by procedures such as described by Gutoff, *Photographic Science and Engineering*, Vol. 14, pages 248-257 (1970), U.S. Pat. Nos. 4,434,226, 4,414,310, 4,433,048 and 4,439,520 and U.K. Patent 2,112,157.

Even if the grains have a uniform crystal structure their interior portions and exterior portions may have different halogen compositions and the grains may also have a lamellar structure. Further, silver halides with different compositions may be bonded by epitaxial bonding and they may be bonded with compounds other than silver halides, e.g., silver thiocyanate or lead oxide.

A mixture of grains with a variety of crystal shapes, may also be used.

A variety of polyvalent metal ion impurities may be introduced into the silver halide emulsion used in the invention during the emulsion grain formation stage or physical ripening stage. Examples of compounds that can be used include salts of cadmium, zinc, copper and thallium, and salts or complex salts of the group VIII elements iron, ruthenium, rhodium, palladium, osmium, iridium and platinum. These group VIII elements are preferred. The amounts of such compounds added extends over a wide range depending on purpose and is suitably  $10^{-9}$  to  $10^{-2}$  moles relative to the silver halide.

Silver halide emulsions are generally used after physical ripening, chemical ripening and spectral sensitization. Additives that are used in these stages are de-

scribed in *Research Disclosure* No. 17643 and No. 18716, listed in the table below.

The two issues of *Research Disclosure* noted above also describe known photographic additives that can be used in the invention, as described in the following table.

|    | Type of Additives                                 | RD 17643              | RD 18716                                         |
|----|---------------------------------------------------|-----------------------|--------------------------------------------------|
| 10 | 1. Chemical Sensitizers                           | Page 23               | Page 648, right column                           |
|    | 2. Speed Enhancers                                |                       | Page 648, right column                           |
|    | 3. Spectral Sensitizers                           | Pages 23 to 24        | Page 648, right column to page 649, right column |
|    | Strong Color                                      |                       |                                                  |
|    | Sensitizers                                       |                       |                                                  |
| 15 | 4. Brightening Agents                             | Page 24               |                                                  |
|    | 5. Antifoggants and Stabilizers                   | Pages 24 to 25        | Page 649, right column                           |
|    | 6. Light-Absorbers, Filter Dyes, UV-Ray Absorbers | Pages 25 to 26        | Page 649, right column to page 650, left column  |
|    | 7. Stain preventives                              | Page 25, right column | Page 650, left column to right column            |
| 20 | 8. Dye Image Stabilizers                          | Page 25               |                                                  |
|    | 9. Hardeners                                      | Page 26               | Page 651, left column                            |
| 25 | 10. Binders                                       | Page 26               | Page 651, left column                            |
|    | 11. Plasticizers, Lubricants                      | Page 27               | Page 650, right column                           |
|    | 12. Coating Assistants, Surfactants               | Pages 26 to 27        | Page 650, right column                           |
| 30 | 13. Antistatic Agents                             | Page 27               | Page 650, right column                           |

A variety of color couplers can be used in the invention. Specific examples of these are described in the patents cited in *Research Disclosure* (RD) No. 17643 VII-C to G.

The couplers disclosed in U.S. Pat. Nos. 3,933,501, 4,022,620, 4,326,024 and 4,401,752, JP-B-58-10739 and U.K. Patents 1,425,020 and 1,476,760 are preferred as yellow couplers.

5-Pyrazolone and pyrazoloazole compounds are preferred as magenta couplers, the materials disclosed in U.S. Pat. Nos. 4,310,619 and 4,351,897, European Patent 73,636, U.S. Pat. Nos. 3,061,432, 3,725,067, *Research Disclosure* No. 24220 (June 1984), JP-A-60-33552, *Research Disclosure* No. 24230 (June 1984), JP-A-60-43659 and U.S. Pat. Nos. 4,500,630, 4,540,654 and 4,556,630 and WO (PCT) 88/04795 being particularly preferred.

Phenolic and naphtholic couplers can be used as cyan couplers, the materials as disclosed in U.S. Pat. Nos. 4,052,212, 4,146,396, 4,228,233, 4,296,200, 2,369,929, 2,801,171, 2,772,162, 2,895,826, 3,772,002, 3,758,308, 4,334,011 and 4,327,173, West German Patent Application (OLS) 3,329,729, European Patent 121,365A, U.S. Pat. Nos. 3,446,622, 4,333,999, 4,451,559, 4,427,767, 4,690,889, 4,254,212 and 4,296,199, European Patent 161,626 and JP-A-61-42658 being preferred.

The colored couplers disclosed in *Research Disclosure* No. 17643 page VII-G, U.S. Pat. No. 4,163,670, JP-B-57-39413, U.S. Pat. Nos. 4,004,929 and 4,138,258 and U.K. Patent 1,146,368 are preferred for correcting unwanted coupling dye absorption.

The materials disclosed in U.S. Pat. No. 4,366,237, U.K. Patent 2,125,570, European Patent 96,570 and West German Patent Application (OLS) 3,234,533 are preferred couplers providing coupling dyes with suitable diffusion characteristics.

Typical examples of polymerized dye-forming couplers are disclosed in U.S. Pat. Nos. 3,451,820, 4,080,211 and 4,367,282 and U.K. Patent 2,102,173.

Couplers which release photographically useful residual groups during coupling also may be suitably employed in the invention. The materials disclosed in the patents noted in RD17643 page VII-F, JP-A-57-151944, JP-A-57-154234 and JP-A-60-184248 and U.S. Pat. No. 4,248,962 are preferred DIR couplers which release development inhibition agents.

The materials disclosed in U.K. Patents 2,097,140 and 2,131,188, JP-A-59-157638 and JP-A-59-70840 are preferred couplers which release nucleating agents in image form or development acceleration agents at the time of development.

Other couplers which may be used in the photosensitive material of the invention include the competing couplers disclosed in U.S. Pat. No. 4,130,427, the polyequivalent couplers disclosed in U.S. Pat. Nos. 4,283,472, 4,338,393 and 4,310,618, the DIR redox compound releasing couplers disclosed in, e.g., JP-A-60-85950 and the couplers disclosed in European Patent 73,302A which release dyes that recolor after elimination.

The couplers used in the invention may be introduced into the photosensitive material by a variety of known dispersion methods.

Examples of high boiling point solvents that can be used in an oil-in-water droplet dispersion method are disclosed in U.S. Pat. No. 2,322,027.

Specific examples of latex dispersion methods and latexes for impregnation are disclosed in U.S. Pat. No. 4,199,363 and West German Patent Applications (OLS) 2,541,274 and 2,541,230.

Preferably the compounds noted below are used together with the couplers in the invention, in particular in combination with pyrazoloazole couplers.

Simultaneous or independent use of a compound (F), shown below, which bonds chemically with an aromatic amine developing agent remaining after color development to form a compound that is chemically inert and essentially colorless and/or a compound (G) which bonds chemically with the oxidation products of aromatic amine color developing agent oxides remaining after color development to form a compound that is chemically inert and essentially colorless is desirable. It prevents stains and other side effects caused by coupler dye formation due to a reaction between couplers and color developing agents or oxidation products thereof remaining in the film in post-processing storage.

Compound (F) is preferably a compound whose secondary reaction rate constant  $k_2$  in reaction with p-anisidine (in 80° C. trioctyl phosphate) is in the range 1.0 l/mol.sec to  $1 \times 10^{-5}$  l/mol.sec. The secondary reaction rate constant can be determined by the method described in JP-A-63-158545.

If  $k_2$  is above this range, the compound itself becomes unstable and may be decomposed through reaction with gelatin or water. On the other hand, if  $k_2$  is below this range, its reaction with residual aromatic amine developing agents is slow and consequently it is not possible to prevent side effects from residual aromatic amine developing agents.

Preferred examples of this compound (F) are represented by formulas (FI) and (FII).

-continued



(FII)

In the formulae,  $\text{R}_1$  and  $\text{R}_2$ , which may be the same or different, each represents aliphatic, aromatic or heterocyclic groups.  $n$  represents 1 or 0. A represents a group which reacts with an aromatic amine developing agent to form a chemical bond, and X represents a group which is eliminated through reaction with an aromatic amine developing agent. B represents hydrogen or an aliphatic, aromatic, heterocyclic, acyl or sulfonyl group; and Y represents a group which accelerates addition of an aromatic amine developing agent to a compound of general formula (FII). A cyclic structure may be formed by bonding of  $\text{R}_1$  with X and Y with  $\text{R}_2$  or B.

20 Typical modes of chemical bonding with the residual aromatic amine developing agent are a substitution reaction and an addition reaction.

The compounds disclosed in, e.g., JP-A-63-15845, JP-A-62-283338 and Japanese Patent Applications 62-158342 and 63-18439 are suitable as specific examples of compounds representable by formulae (FI) and (FII).

Preferred examples of compound (G) which bonds chemically with the oxidation products of residual aromatic amine developing agent to form a chemically inert, colorless compound after color development processing are represented by formula (GI):



35 In the formula, R represents an aliphatic group, aromatic residue or heterocyclic group. Z represents a nucleophilic group or a group which is decomposed in the photosensitive material after development and releases a nucleophilic group. The compound represented by formula (GI) is preferably one in which Z is a group having a Pearson's nucleophilicity  $^n\text{CH}_3$  value (R. G. Pearson et al., *J. Am. Chem. Soc.*, 90, 319 (1968)) of 5 or more, or is a group derived from such a group.

40 The compounds disclosed in, e.g., European Patent Application (OPI) 255722, JP-A-62-143048, JP-A-62-229145 and Japanese Patent Applications 63-18439, 63-136724, 62-214681 and 62-158342 are suitable as specific examples of compounds represented by formula (GI).

45 50 Suitable combinations of compound (G) and compound (F) are described in Japanese Patent Application 63-18439.

55 Supports suitable for use in the invention are described in, RD No. 17643, page 28 and No. 18716, page 647 right-hand column to page 648 left-hand column.

60 65 The photosensitive material to which the invention is applied may be any color photographic photosensitive material such as, e.g., a color negative film, color reversal film (internal type or external type), color paper, color positive film, color reversal paper, color diffusion transfer process material and direct positive color photosensitive material, but its use for color negative film, color reversal film and color transfer paper is particularly preferred.

66 The present invention is now illustrated in greater detail with reference to the following specific examples, but the present invention is not to be construed as being

limited thereto. Unless otherwise indicated, all part, percents and ratios are by weight.

## EXAMPLE 1

A multilayer color printing paper with the layer structure described below was prepared on a paper support laminated on both sides with polyethylene. The coating solutions were prepared as follows.

## Preparation of 1st Layer Coating Solution

60.0 g of a yellow coupler (ExY) and 28.0 g of a fading preventive (Cpd-1) were dissolved by addition of 150 cc of ethyl acetate, 1.0 cc of a solvent (Solv-3) and 3.0 cc of another solvent (Solv-4). To this solution was added 450 cc of a 10% gelatin aqueous solution containing sodium dodecylbenzenesulfonate and then dispersion was effected in an ultrasonic homogenizer and the resulting dispersion was mixed with and dissolved in 420 g of a silver chlorobromide emulsion (silver bromide 0.7 mol %) containing the blue sensitization dye described below, providing the 1st layer coating solution. The coating solution of the 2nd to 7th layers were prepared in the same manner. 1,2-Bis(vinylsulfonyl)ethane was used as a gelatin hardener for each layer.

The following substances were used as the spectral sensitization dyes for the various layers.

## Blue-sensitive Emulsion Layer

Anhydro-5-5'-chloro-3,3'-disulfoethylthiacyanine hydroxide

## Green-sensitive Emulsion Layer

Anhydro-9-ethyl-5,5'-diphenyl-3,3'-disulfoethyloxacarbocyanine hydroxide

## Red-sensitive Emulsion Layer

3,3'-diethyl-5-methoxy-9,9'-(2,2'-dimethyl-1,3-propano)thiadicarbocyanine iodide

The following material was used as a stabilizer for each layer.

|                                              |   |                       |
|----------------------------------------------|---|-----------------------|
| 1-(2-acetoaminophenyl)-5-mercaptopetetrazole | 7 | Mixture (molar ratio) |
| 1-phenyl-5-mercaptopetetrazole               | 2 |                       |
| 1-(p-methoxyphenyl)-5-mercaptopetetrazole    | 1 |                       |

The following substances were used as antiirradiation dyes.

[3-carboxy-5-hydroxy-4-(3-(3-carboxy-5-oxo-1-(2,5-disulfonatophenyl)-2-pyrazolin-1-hydrazolyl)benzene-2,5-disulfonate, disodium salt  
N,N'-(4,8-dihydroxy-9,10-dioxo-3,7-disulfonatoanthracene-1,5-diyl)bis(aminomethanesulfonat), tetrasodium salt  
3-cyano-5-hydroxy-4-(3-(3-cyano-5-oxo-1-(4-sulfonatophenyl)-2-pyrazoline-4-ylidene)-1-pentanyl)-1-pyralolyl]benzene-4-sulfonate, sodium salt

## Layer Structure

The compositions of the various layers are described below. The figures indicate coating quantities (g/m<sup>2</sup>). Coating quantities calculated as silver are given for silver halide emulsions.

## Support

Paper support - laminated on both sides with polyethylene

|                                                                                  |       |
|----------------------------------------------------------------------------------|-------|
| <u>1st Layer: Blue-sensitive Layer</u>                                           |       |
| Silver halide emulsion (AgBr: 0.7 mol %, cubic, average grain size 0.9 $\mu$ m)  | 0.27  |
| Gelatin                                                                          | 1.80  |
| Yellow coupler (ExY)                                                             | 0.60  |
| Fading preventive (Cpd-1)                                                        | 0.28  |
| Solvent (Solv-3)                                                                 | 0.01  |
| Solvent (Solv-4)                                                                 | 0.03  |
| <u>2nd Layer: Color-mixing Prevention Layer</u>                                  |       |
| Gelatin                                                                          | 0.80  |
| Color-mixing preventive (Cpd-2)                                                  | 0.055 |
| Solvent (Solv-1)                                                                 | 0.03  |
| Solvent (Solv-2)                                                                 | 0.015 |
| <u>3rd Layer: Green-sensitive Layer</u>                                          |       |
| Silver halide emulsion (AgBr: 0.7 mol %, cubic, average grain size 0.45 $\mu$ m) | 0.28  |
| Gelatin                                                                          | 1.40  |
| Magenta coupler (ExM)                                                            | 0.67  |
| Fading preventive (Cpd-3)                                                        | 0.23  |
| Fading preventive (Cpd-4)                                                        | 0.11  |
| Solvent (Solv-1)                                                                 | 0.20  |
| Solvent (Solv-2)                                                                 | 0.02  |
| <u>4th Layer: Color-mixing Prevention Layer</u>                                  |       |
| Gelatin                                                                          | 1.70  |
| Color-mixing preventive (Cpd-2)                                                  | 0.065 |
| Ultraviolet ray absorber (UV-1)                                                  | 0.45  |
| Ultraviolet ray absorber (UV-2)                                                  | 0.23  |
| Solvent (Solv-1)                                                                 | 0.05  |
| Solvent (Solv-2)                                                                 | 0.05  |
| <u>5th Layer: Red-sensitive Layer</u>                                            |       |
| Silver halide emulsion (AgBr: 0.7 mol %, cubic, average grain size 0.5 $\mu$ m)  | 0.19  |
| Gelatin                                                                          | 1.80  |
| Cyan coupler (ExC-1)                                                             | 0.26  |
| Cyan coupler (ExC-2)                                                             | 0.12  |
| Fading preventive (Cpd-1)                                                        | 0.20  |
| Solvent (Solv-1)                                                                 | 0.16  |
| Solvent (Solv-2)                                                                 | 0.09  |
| <u>6th Layer: Ultraviolet Absorption Layer</u>                                   |       |
| Gelatin                                                                          | 0.70  |
| Ultraviolet absorber (UV-1)                                                      | 0.26  |
| Ultraviolet absorber (UV-2)                                                      | 0.07  |
| Solvent (Solv-1)                                                                 | 0.30  |
| Solvent (Solv-2)                                                                 | 0.09  |
| <u>7th Layer: Protective Layer</u>                                               |       |
| Gelatin                                                                          | 1.07  |

The compounds used were as follows:

- (ExY) Yellow coupler  
 $\alpha$ -pivaroyl- $\alpha$ -(3-benzyl-1-hydantoinyl)-2-chloro-5-[ $\beta$ -dodecylsulfonyl]-butylamido]acetoinilide  
 (ExM) Magenta coupler  
 1-(2,4,6-trichlorophenyl-3[2-chloro-5-(3-octadecenyl-succinimido)anilino]-5-pyrazolone  
 (ExC-1) Cyan coupler  
 2-Pentafluorobenzamido-4-chloro-5-[2-(2,4-di-tert-amyloxy)-3-methylbutylamido]phenol  
 (ExC-2) Cyan coupler  
 2,4-dichloro-3-methyl-6-[ $\alpha$ -2,4-di-tert-amyloxy]-butylamido]phenol  
 (Cpd-1) Color-fading preventive  
 2,5-di-tert-amylophenyl-3,5-di-tert-butylhydroxy benzoate  
 (Cpd-2) Color-mixing preventive  
 2,5-di-tert-octylhydroquinone  
 (Cpd-3) Color-fading preventive  
 1,4-di-tert-amylo-2,5-di-tert-butyloxybenzene  
 (Cpd-4) Color-fading preventive  
 2,2'-methylenebis(4-methyl-6-tert-butylphenol)

(Cpd-5)  
p-(p-toluenesulfonamido)phenyldodecane  
(Solv-3) Solvent

(B-11) Solvent

### **(Solv-4) Solvent**

### (Solv.) Solvent

## 14,14-Dicyanobiphenyl

### **(UV-1) Ultraviolet absorber**

(3V-1)  $\oplus$

(IV-2) Ultraviolet-ray absorption

### (UV-2) Ultraviolet ray absorber

**2-(2-hydroxy-3,5-di-tert-butyl (Solv. 1) Solvent**

**(Solv-1) Solvent**

### Di-(2-ethylhexyl) Sulfoxide

**(Solv-2) Solvent**

### Dibutyl phthalate

The sample material prepared in the manner indicated above was designated as A. Samples B to E were prepared by making the changes noted in Table 1 to the emulsion silver halide compositions.

TABLE 1

| Sample | Emulsion Silver Halide Composition<br>(Cl content mol %) |      |    |
|--------|----------------------------------------------------------|------|----|
|        | BL                                                       | GL   | RL |
| A      | 99.3                                                     | 99.3 | 98 |
| B      | 95                                                       | 95   | 95 |
| C      | 80                                                       | 80   | 80 |
| D      | 70                                                       | 70   | 70 |
| E      | 50                                                       | 50   | 50 |

The following tests were conducted in order to investigate the photographic characteristics of these coating samples.

First, the coating samples were subjected to graduated exposure for sensitometry using a sensitometer (FWH model manufactured by Fuji Photo Film KK, light source color temperature 3200° K.). This was effected at exposures of 250 CMS for 1/10 second

The coating samples were processed in an automatic development machine by the processing stages and processing solutions noted below. The composition of the color development solution was varied in the manner indicated in Table 2.

| Processing Stage  | Temperature | Time       |
|-------------------|-------------|------------|
| Color development | 38° C.      | 45 seconds |
| Bleach-fix        | 30-36° C.   | 45 seconds |
| Rinse (1)         | 30-37° C.   | 30 seconds |
| Rinse (2)         | 30-37° C.   | 30 seconds |
| Rinse (3)         | 30-37° C.   | 30 seconds |
| Drying            | 70-80° C.   | 60 seconds |

The compositions of the various processing solutions were as follows.

| <u>Color Development Solution</u> |                                                      |
|-----------------------------------|------------------------------------------------------|
| 5                                 | Water 800 ml                                         |
|                                   | Ethylenediamine-N,N,N,N,-tetra- 3.0 g                |
|                                   | methyleneephosphonic acid                            |
|                                   | Organic preservative A (I-1) 0.03 mol                |
|                                   | Sodium chloride See Table 2                          |
| 10                                | Potassium bromide See Table 2                        |
|                                   | Potassium carbonate 25 g                             |
|                                   | N-ethyl-N-( $\beta$ -methanesulfonamidoethyl)- 5.0 g |
|                                   | 3-methyl-4-aminoaniline sulfite                      |
|                                   | Triethanolamine 10.0 g                               |
|                                   | Brightening agent (4,4'-diaminostilbene 2.0 g        |
|                                   | based)                                               |
| 15                                | Sodium sulfite 0.1 g                                 |
|                                   | Water added 1000 ml                                  |
|                                   | pH (25° C.) 10.05                                    |
| <u>Bleach-fix Solution</u>        |                                                      |
|                                   | Water 400 ml                                         |
| 20                                | Ammonium thiosulfate (70%) 100 ml                    |
|                                   | Sodium sulfite 17 g                                  |
|                                   | Ferric(III) ammonium ethylene- 55 g                  |
|                                   | diaminetetraacetate                                  |
|                                   | Disodium ethylenediaminetetraacetate 5 g             |
|                                   | Ammonium bromide 40 g                                |
|                                   | Glacial acetic acid 9 g                              |
| 25                                | Water added 1000 ml                                  |
|                                   | pH (25° C.) 5.40                                     |

### Rinse Solution

Ion exchange water (both calcium and magnesium each not more than 3 ppm)

The blue (B), green (G) and red (R) maximum densities ( $D_{max}$ ) achieved in the sensitometry described above were measured by means of a Macbeth densitometer. The results are shown in Table 2.

The coating samples were also subjected to exposure to uniform grey light using a sensitometer (FWH model manufactured by Fuji Photo Film KK, light source color temperature 3200° K.) and processed in the same way as described above, and assessment of sensitization streaks was made. The assessment standards were in 4 stages, as follows.

| 45 | Sensitization<br>Streak Assessment | Number of Sensitization Streaks in<br>100 cm <sup>2</sup> (10 cm × 10 cm) of Sample |
|----|------------------------------------|-------------------------------------------------------------------------------------|
|    | ○                                  | 0                                                                                   |
|    | △                                  | 1-2                                                                                 |
|    | x                                  | 3-5                                                                                 |
|    | xx                                 | 6 or more                                                                           |

TABLE 2

TABLE 2-continued

| Streaks                            |                            | 9                          | 10                         | 11                         | 12                         | 13                         | 14                         | 15                         | 16                         | 17                         |
|------------------------------------|----------------------------|----------------------------|----------------------------|----------------------------|----------------------------|----------------------------|----------------------------|----------------------------|----------------------------|----------------------------|
| Processing Example                 |                            | A                          | B                          | C                          | D                          | E                          | D                          | D                          | D                          | D                          |
| Coating Sample Development         |                            | $3.0 \times 10^{-1}$       | $3.0 \times 10^{-1}$       | 0                          | $1.0 \times 10^{-1}$       | $1.0 \times 10^{-1}$       | 0                          | $3.5 \times 10^{-2}$       | $1.5 \times 10^{-1}$       | $3.0 \times 10^{-1}$       |
| Solution                           |                            |                            |                            |                            |                            |                            |                            |                            |                            |                            |
| Chloride Ion Concentration (mol/l) |                            | $5.0 \times 10^{-3}$       | $1.0 \times 10^{-6}$       | 0                          | $1.0 \times 10^{-3}$       | $1.0 \times 10^{-3}$       | 0                          | $3.0 \times 10^{-5}$       | $1.0 \times 10^{-3}$       | $5.9 \times 10^{-3}$       |
| Development Solution               |                            |                            |                            |                            |                            |                            |                            |                            |                            |                            |
| Bromide Ion Concentration (mol/l)  |                            |                            |                            |                            |                            |                            |                            |                            |                            |                            |
| Remarks                            | Compar-<br>ison<br>Example | Compar-<br>ison<br>Example | Compar-<br>ison<br>Example | Compar-<br>ison<br>Example | Compar-<br>ison<br>Example | Compar-<br>ison<br>Example | Compar-<br>ison<br>Example | Compar-<br>ison<br>Example | Compar-<br>ison<br>Example | Compar-<br>ison<br>Example |
| BL (D <sub>max</sub> )             | 1.90                       | 2.01                       | 2.38                       | 1.69                       | 1.38                       | 1.72                       | 1.70                       | 1.69                       | 1.63                       | 1.63                       |
| GL (D <sub>max</sub> )             | 2.23                       | 2.29                       | 2.49                       | 2.01                       | 1.98                       | 2.08                       | 2.05                       | 2.00                       | 2.00                       | 2.00                       |
| RL (D <sub>max</sub> )             | 2.76                       | 2.80                       | 2.96                       | 2.58                       | 2.39                       | 2.62                       | 2.60                       | 2.56                       | 2.50                       | 2.50                       |
| Sensitization Streaks              | ○                          | xx                         | xx                         | Δ                          | Δ                          | Δ                          | Δ                          | Δ                          | Δ                          | Δ                          |

It is apparent from Table 2 that in processing examples 1 to 6 in which the photosensitive materials A to C of the invention were processed with development solutions of the invention, the maximum density was high and occurrence of sensitization streaks was prevented.

In processing example 9, sensitization streaks were prevented but the maximum density was low and rapid development was not achieved. In processing examples 7, 8, 10 and 11, the maximum density was high but sensitization streaks occurred.

With processing examples 12 to 17, there was less occurrence of sensitization streaks but the maximum density was low and again rapid development processing was not achieved. As seen in examples 12 and 14 to 17, when use was made of a photosensitive material whose silver chloride content is less than 80 mol % there was hardly any change in occurrence of pressure sensitization streaks or the maximum density, regardless of whether the chlorine ion and bromine ion concentration were within the ranges of the invention or not. As seen in processing examples 1 to 11, when a high silver chloride photosensitive material was used the characteristic maximum density and prevention of sensitization streaks were achieved only when the chlorine ion and bromine ion concentrations were within the ranges of the invention.

#### EXAMPLE 2

A multilayer color printing paper with the layer structure described below was prepared on a paper

support laminated on both sides with polyethylene. The coating solutions were prepared as follows.

#### Preparation of 1st layer coating solution

19.1 g of a yellow coupler (E×Y), 4.4 g of a color image stabilizer (Cpd-1) and 0.7 g of another color image stabilizer (Cpd-7) were dissolved by addition of 27.2 cc of ethyl acetate and 8.2 g of a solvent (Solv-3). This solution was emulsified and dispersed in 185 cc of a 10% gelatin aqueous solution containing 8 cc of sodium dodecylbenzenesulfonate. Meanwhile, an emulsion was produced by adding to a silver chlorobromide emulsion (average cubic grain size 0.85 μm, cubic grains with a grain size distribution variation coefficient of 0.07 and containing locally present 1.0 mol % silver bromide in some parts on grain surfaces) the two types of blue-sensitization dyes described below in an amount that was  $2.0 \times 10^{-4}$  moles per 1 mole of silver in each case, and effecting sulfur sensitization. This emulsion and the emulsified dispersion described above were mixed and dissolved to give a 1st coating solution with the composition noted below. The coating solutions of the 2nd to 7th layers were prepared in the same manner. 1-oxy-3,5-dichloro-s-triazine sodium salt was used as a gelatin hardener for each layer.

The following substances were used as spectral sensitization dyes in the various layers.

#### Blue-sensitive emulsion layer



( $2.0 \times 10^{-4}$  moles of each of the above 2 types per 1 mole of silver halide)

-continued

Green-sensitive emulsion layer

 $(4.0 \times 10^{-4}$  moles per 1 mole of silver halide)

and

 $(7.0 \times 10^{-5}$  moles per 1 mole of silver halide)

Red-sensitive emulsion layer

 $(0.9 \times 10^{-4}$  moles per 1 mole of silver halide)

The following compound was added to the red-sensitive emulsion layer in an amount that was  $2.6 \times 10^{-3}$  moles per 1 mole of silver halide.

Also, to the blue-sensitive emulsion layer, green-sensitive emulsion layer and red-sensitive emulsion layer were added 1-(5-methylureidophenyl)-5-mercaptopetetrazole in amounts that were respectively  $8.5 \times 10^{-5}$  moles,  $7.7 \times 10^{-4}$  moles and  $2.5 \times 10^{-5}$  moles per 1 mole of silver halide.

The following dyes were added to the emulsion layers to prevent irradiation.



and

-continued



15

## Layer Structure

The figures indicate coating quantities (g/m<sup>2</sup>). Coating quantities calculated as silver are given for silver 20 halide emulsions.

## Support

Polyethylene-laminated paper.

(The polyethylene on the 1st layer side contained a 25 white pigment (TiO<sub>2</sub>) and a blue dye (ultramarine).)

| 1st Layer: Blue-sensitive Layer                                                                                                                                                               |      |    |
|-----------------------------------------------------------------------------------------------------------------------------------------------------------------------------------------------|------|----|
| The silver chlorobromide emulsion described above                                                                                                                                             | 0.30 | 30 |
| Gelatin                                                                                                                                                                                       | 1.86 |    |
| Yellow coupler (ExY)                                                                                                                                                                          | 0.82 |    |
| Color image stabilizer (Cpd-1)                                                                                                                                                                | 0.19 |    |
| Color image stabilizer (Cpd-7)                                                                                                                                                                | 0.03 |    |
| Solvent (Solv-3)                                                                                                                                                                              | 0.35 | 35 |
| 2nd Layer: Color-mixing Prevention Layer                                                                                                                                                      |      |    |
| Gelatin                                                                                                                                                                                       | 0.99 |    |
| Color-mixing preventive (Cpd-5)                                                                                                                                                               | 0.08 |    |
| Solvent (Solv-1)                                                                                                                                                                              | 0.16 |    |
| Solvent (Solv-4)                                                                                                                                                                              | 0.08 |    |
| 3rd Layer: Green-sensitive Layer                                                                                                                                                              |      |    |
| Silver chlorobromide emulsion (cubic grain size 0.40 μm, grain size distribution variation coefficient 0.09, includes locally present 1 mol % silver bromide in some parts on grain surfaces) | 0.20 | 40 |
| Gelatin                                                                                                                                                                                       | 1.24 |    |
| Magenta coupler (ExM)                                                                                                                                                                         | 0.29 |    |

-continued

|                                                                                                                                                                                                 |      |
|-------------------------------------------------------------------------------------------------------------------------------------------------------------------------------------------------|------|
| Color image stabilizer (Cpd-3)                                                                                                                                                                  | 0.09 |
| Color image stabilizer (Cpd-4)                                                                                                                                                                  | 0.06 |
| Solvent (Solv-2)                                                                                                                                                                                | 0.32 |
| Solvent (Solv-7)                                                                                                                                                                                | 0.16 |
| <u>4th Layer: Ultraviolet Absorption Layer</u>                                                                                                                                                  |      |
| Gelatin                                                                                                                                                                                         | 1.58 |
| Ultraviolet ray absorber (UV-1)                                                                                                                                                                 | 0.47 |
| Color-mixing preventive (Cpd-5)                                                                                                                                                                 | 0.05 |
| Solvent (Solv-5)                                                                                                                                                                                | 0.24 |
| <u>5th Layer: Red-sensitive Layer</u>                                                                                                                                                           |      |
| Silver chlorobromide emulsion (cubic grain size 0.36 μm, grain size distribution variation coefficient 0.11, includes locally present 1.6 mol % silver bromide in some parts on grain surfaces) | 0.21 |
| Gelatin                                                                                                                                                                                         | 1.34 |
| Cyan coupler (ExC)                                                                                                                                                                              | 0.34 |
| Color image stabilizer (Cpd-6)                                                                                                                                                                  | 0.17 |
| Color image stabilizer (Cpd-7)                                                                                                                                                                  | 0.34 |
| Color image stabilizer (Cpd-9)                                                                                                                                                                  | 0.04 |
| Solvent (Solv-4)                                                                                                                                                                                | 0.37 |
| <u>6th Layer: Ultraviolet Absorption Layer</u>                                                                                                                                                  |      |
| Gelatin                                                                                                                                                                                         | 0.53 |
| Ultraviolet ray absorber (UV-1)                                                                                                                                                                 | 0.16 |
| Color-mixing preventive (Cpd-5)                                                                                                                                                                 | 0.02 |
| Solvent (Solv-5)                                                                                                                                                                                | 0.08 |
| <u>7th Layer: Protective Layer</u>                                                                                                                                                              |      |
| Gelatin                                                                                                                                                                                         | 1.33 |
| Acryl-modified polyvinyl alcohol copolymer (modification degree 17%)                                                                                                                            | 0.17 |
| Liquid paraffin                                                                                                                                                                                 | 0.03 |

The following compounds were used.

## (ExY) Yellow coupler



## (ExM) Magenta coupler

-continued



### (ExC) Cyan coupler

A 1:3:6 mixture (by weight) of the following compounds,

wherein R = H; R = C<sub>2</sub>H<sub>5</sub>; R = C<sub>4</sub>H<sub>9</sub>.



**(Cpd-1) Color image stabilizer**



**(Cpd-3) Color image stabilizer**



**(Cpd-4) Color image stabilizer**



**(Cpd-5) Color mixing preventive**

-continued



(Cpd-6) Color image stabilizer  
2:4:4 mixture (by weight) of (A):(B):(C)



(Cpd-7) Color image stabilizer



Average molecular weight 60,000

(Cpd-9) Color mixing preventive



(UV-1) Ultraviolet absorbent  
4:2:4 mixture (by weight) of (D):(E):(F)



(Solv-1) Solvent



(Solv-2) Solvent  
3:7 mixture (by weight) of

-continued



(Solv-3) Solvent  
 $O=P-\text{O}-\text{C}_9\text{H}_{19}(\text{iso})_3$

(Solv-4) Solvent



(Solv-5) Solvent  
 $\text{COOC}_8\text{H}_{17}$   
 $(\text{CH}_2)_8$   
 $\text{COOC}_8\text{H}_{17}$

(Solv-6) Solvent



The sample material prepared in the manner indicated above was designated as F.

The following tests were conducted in order to investigate the photographic characteristics of this coating material F.

First, the coating material was subjected to graduated exposure for sensitometry using a sensitometer (FWH model manufactured by Fuji Photo Film Co., Ltd., light source color temperature 3200° K.). This was effected at exposures of 250 CMS for 1/10 second.

The coating material was processed in an automatic development machine by the processing stages and processing solutions noted below. The composition of the color development solution was varied in the manner indicated in Table 3.

| Processing Stage  | Temperature | Time       |
|-------------------|-------------|------------|
| Color development | 38° C.      | 45 seconds |
| Bleach-fix        | 30-36° C.   | 45 seconds |
| Rinse (1)         | 30-37° C.   | 30 seconds |
| Rinse (2)         | 30-37° C.   | 30 seconds |
| Rinse (3)         | 30-37° C.   | 30 seconds |
| Drying            | 70-80° C.   | 60 seconds |

The compositions of the various processing solutions were as follows.

| Color Development Solution                                                     |             |
|--------------------------------------------------------------------------------|-------------|
| Water                                                                          | 800 ml      |
| Ethylenediamine-N,N,N,N-tetramethyleneephosphonic acid                         | 3.0 g       |
| Organic preservative A (See Table 3)                                           | 0.03 mol    |
| Sodium chloride                                                                | See Table 3 |
| Potassium bromide                                                              | See Table 3 |
| Potassium carbonate                                                            | 25 g        |
| N-ethyl-N-( $\beta$ -methanesulfonamidoethyl)-3-methyl-4-aminonaniline sulfite | 5.0 g       |
| Triethanolamine                                                                | 10.0 g      |
| Brightening agent (4,4'-diaminostilbene based)                                 | 2.0 g       |
| Sodium sulfite                                                                 | 0.1 g       |
| Water added                                                                    | 1000 ml     |
| pH (25° C.)                                                                    | 10.05       |
| Bleach-fix Solution                                                            |             |
| Water                                                                          | 400 ml      |
| Ammonium thiosulfate (70%)                                                     | 100 ml      |
| Sodium sulfite                                                                 | 17 g        |
| Ferric(III) ammonium ethylenediaminetetraacetate                               | 55 g        |
| Disodium ethylenediaminetetraacetate                                           | 5 g         |
| Ammonium bromide                                                               | 40 g        |
| Glacial acetic acid                                                            | 9 g         |
| Water added                                                                    | 1000 ml     |
| pH (25° C.)                                                                    | 5.40        |

## Rinse Solution

Ion exchange water (both calcium and magnesium not more than 3 ppm)

Sensitometry processing as described above was effected and the blue (B) minimum density ( $D_{min}$ ) and maximum density ( $D_{max}$ ) were measured by means of a Macbeth densitometer. The results are shown in Table 3.

Sensitometry was similarly performed after the above development solution had been left to age for 2 weeks at room temperature open to air with an opening ratio (opening area/solution volume) of  $0.02 \text{ cm}^{-1}$ . The changes in the blue (B) minimum density that occurred over the period were determined by means of a Macbeth densitometer, as shown in Table 3.

The aged color development solution was also used for assessments of sensitization streaks as in Example 1. The assessment standards were in 4 stages, as follows.

| Sensitization Streak Assessment | Number of Sensitization Streaks in $100 \text{ cm}^2$ ( $10 \text{ cm} \times 10 \text{ cm}$ ) of Sample |
|---------------------------------|----------------------------------------------------------------------------------------------------------|
| ○                               | 0                                                                                                        |
| △                               | 1-2                                                                                                      |
| ×                               | 3-5                                                                                                      |
| xx                              | 6 or more                                                                                                |

TABLE 3

| Processing I Example                     | 1                    | 2                    | 3                    | 4                    | 5                    | 6                    |
|------------------------------------------|----------------------|----------------------|----------------------|----------------------|----------------------|----------------------|
| Development Solution                     | $3.5 \times 10^{-2}$ | $5.0 \times 10^{-2}$ | $1.0 \times 10^{-2}$ | $1.5 \times 10^{-2}$ | $1.0 \times 10^{-2}$ | $1.0 \times 10^{-2}$ |
| Chloride Ion Concentration (mole/l)      |                      |                      |                      |                      |                      |                      |
| Development Solution                     | $3.0 \times 10^{-5}$ | $5.0 \times 10^{-5}$ | $4.0 \times 10^{-4}$ | $1.0 \times 10^{-3}$ | $4.0 \times 10^{-4}$ | $4.0 \times 10^{-4}$ |
| Bromide Ion Concentration (mole/l)       |                      |                      |                      |                      |                      |                      |
| Organic Preservative A                   | I-1                  | I-1                  | I-1                  | I-1                  | II-19                |                      |
| Remarks                                  | Invention            | Invention            | Invention            | Invention            | Invention            | Invention            |
| BL $D_{max}$ (Before aging)              | 2.48                 | 2.48                 | 2.47                 | 2.40                 | 2.53                 | 2.36                 |
| BL $D_{min}$ (After aging)               | 0.07                 | 0.07                 | 0.07                 | 0.07                 | 0.07                 | 0.08                 |
| BL $\Delta D_{min}$ (Before/after aging) | +0.01                | $\pm 0.00$           | $\pm 0.00$           | $\pm 0.00$           | $\pm 0.00$           | +0.02                |
| Sensitization Streaks                    | ○                    | ○                    | ○                    | ○                    | ○                    | - △                  |
| Processing I Example                     | 7                    | 8                    | 9                    | 10                   | 11                   | 12                   |
| Development Solution                     | —                    | $1.0 \times 10^{-2}$ | —                    | $5.0 \times 10^{-2}$ | $3.0 \times 10^{-1}$ | $1.0 \times 10^{-1}$ |
| Chloride Ion Concentration (mole/l)      |                      |                      |                      |                      |                      |                      |
| Development Solution                     | —                    | —                    | $4.0 \times 10^{-4}$ | $5.0 \times 10^{-3}$ | $5.0 \times 10^{-4}$ | $1.0 \times 10^{-2}$ |
| Bromide Ion Concentration (mole/l)       |                      |                      |                      |                      |                      |                      |
| Organic Preservative A                   | I-1                  | I-1                  | I-1                  | I-1                  | I-1                  | I-1                  |
| Remarks                                  | Comparison Example   | Comparison Example   | Comparison Example   | Comparison Example   | Comparison Example   | Comparison Example   |
| BL $D_{max}$ (Before aging)              | 2.49                 | 2.48                 | 2.48                 | 1.94                 | 2.16                 | 1.70                 |
| BL $D_{min}$ (After aging)               | 0.14                 | 0.13                 | 0.10                 | 0.07                 | 0.07                 | 0.07                 |
| BL $\Delta D_{min}$ (Before/after aging) | +0.06                | +0.05                | +0.04                | $\pm 0.00$           | +0.01                | $\pm 0.00$           |
| Sensitization Streaks                    | xx                   | xx                   | xx                   | ○                    | △                    | ○                    |

It is seen from Table 3 that in processing examples 1 to 6 in which processing was effected with development solutions of the invention, there were excellent photographic characteristics, since the maximum density was high and the minimum density was low and there was

marked suppression of occurrence of sensitization streaks.

It is also seen that there was marked suppression of increase in the minimum density, and suppression of fluctuation of photographic characteristics even with aging of the color development solution.

Further, in comparison with use of hydroxylamine, which is popular as an organic preservative for developing agents for silver chlorobromide photosensitive materials, use of the organic preservatives I-1 and II-19 was superior since it resulted in only a small change of the minimum density with aging of a development solution, and was also very effective in preventing occurrence of sensitization streaks.

As seen in processing examples 6 to 12, if the chloride ion and bromide ion concentrations were lower than the concentrations of the invention, although the maximum density was high the minimum density also was high and an increase in the minimum density and occurrence

of pressure sensitization streaks accompanying aging of the development solution occurred. If the chlorine ion and bromine ion concentrations were higher than the concentrations of the invention, the minimum density was low and occurrence of pressure sensitization streaks was prevented but the maximum density was low, which means that these concentrations were unsuitable for rapid processing.

## EXAMPLE 3

The procedure in Example 2 was followed, except that in processing example 5, I-2, I-3, II-1, II-5, II-9, II-13 and II-20 were used instead of organic preservative A II-19. Similarly good results were obtained.

#### EXAMPLE 4

The procedure in Example 2 was followed, except that in processing example 5, III-3, III-11, IV-1 and IV-2 were used instead of triethanolamine in the development solution. Similarly good results were obtained.

### EXAMPLE 5

A multilayer color printing paper with the layer structure described below was prepared on a paper support laminated on both sides with polyethylene. The coating solutions were prepared as follows.

### Preparation of 1st Layer Coating Solution

19.1 g of a yellow coupler (E $\times$ Y), 4.4 g of a color image stabilizer (Cpd-1) and 0.7 g of another color image stabilizer (Cpd-7) were dissolved by addition of 27.2 cc of ethyl acetate and 8.2 g of a solvent (Solv-3). This solution was emulsified and dispersed in 185 cc of

5 a 10% gelatin aqueous solution containing 8 cc of 10% sodium dodecylbenzenesulfonate. Meanwhile, an emulsion was produced by adding to a silver chlorobromide emulsion (average cubic grain size 0.85  $\mu\text{m}$ , cubic grains  
 10 with a grain size distribution variation coefficient of 0.07 and having locally present 1.0 mol % silver bromide in some parts on grain surfaces) the two types of blue-sensitization dyes described below, in an amount that was  $2.0 \times 10^{-4}$  moles per 1 mole of silver in each case, and effecting sulfur sensitization. This emulsion and the emulsified dispersion described above were mixed and dissolved to give a 1st coating solution with the composition noted below. The coating solutions of the 2nd to 7th layers were prepared in the same manner.  
 15 1-oxy-3,5-dichloro-s-triazine sodium salt was used as a gelatin hardener for each layer.

The following substances were used as spectral sensitization dyes in the various layers.

### Blue-sensitive emulsion layer



( $2.0 \times 10^{-4}$  moles of each of the above 2 types per 1 mole of silver halide)

### Green-sensitive emulsion layer



( $4.0 \times 10^{-4}$  moles per 1 mole of silver halide)

and



( $7.0 \times 10^{-5}$  moles per 1 mole of silver halide)

### Red-sensitive emulsion layer



( $0.9 \times 10^{-4}$  moles per 1 mole of silver halide)

The following compound was added to the red-sensitive emulsion layer in an amount that was  $2.6 \times 10^{-3}$  moles per 1 mole of silver halide.



Also, to the blue-sensitive emulsion layer, green sensitive emulsion layer and red-sensitive emulsion layer were added 1-(5-methylureidophenyl)-5-mercaptopotetrazole in amounts that were respectively  $8.5 \times 10^{-5}$  moles,  $7.7 \times 10^{-4}$  moles and  $2.5 \times 10^{-5}$  moles per 1 mole of silver halide.

The following dyes were added to the emulsion layers to prevent irradiation.



and



#### Layer Structure

The compositions of the various layers were as follows.

The figures indicate coating quantities (g/m<sup>2</sup>). Coating quantities calculated as silver are given for silver halide emulsions.

#### Support

Polyethylene-laminated paper.

(The polyethylene on the 1st layer side contained a white pigment (TiO<sub>2</sub>) and a blue dye (ultramarine).)

#### 1st Layer: Blue-sensitive Layer

The silver chlorobromide emulsion described above  
Gelatin  
Yellow coupler (ExY)

60

65

-continued

|                                                                                                                                                                                       |      |
|---------------------------------------------------------------------------------------------------------------------------------------------------------------------------------------|------|
| Color image stabilizer (Cpd-1)                                                                                                                                                        | 0.19 |
| Color image stabilizer (Cpd-7)                                                                                                                                                        | 0.03 |
| Solvent (Solv-3)                                                                                                                                                                      | 0.35 |
| <u>2nd Layer: Color-mixing Prevention Layer</u>                                                                                                                                       |      |
| Gelatin                                                                                                                                                                               | 0.99 |
| Color-mixing preventive (Cpd-5)                                                                                                                                                       | 0.08 |
| Solvent (Solv-1)                                                                                                                                                                      | 0.16 |
| Solvent (Solv-4)                                                                                                                                                                      | 0.08 |
| <u>3rd Layer: Green-sensitive Layer</u>                                                                                                                                               |      |
| Silver chlorobromide emulsion<br>(cubic grain size 0.40 $\mu\text{m}$ , variation coefficient 0.09, including locally present 1 mol % silver bromide in some parts on grain surfaces) | 0.36 |
| Gelatin                                                                                                                                                                               | 1.24 |
| Magenta coupler (ExM)                                                                                                                                                                 | 0.31 |
| Color image stabilizer (Cpd-3)                                                                                                                                                        | 0.12 |
| Color image stabilizer (Cpd-4)                                                                                                                                                        | 0.06 |
| Color image stabilizer (Cpd-8)                                                                                                                                                        | 0.09 |
| Solvent (Solv-2)                                                                                                                                                                      | 0.42 |
| <u>4th Layer: Ultraviolet Absorption Layer</u>                                                                                                                                        |      |
| Gelatin                                                                                                                                                                               | 0.58 |
| Ultraviolet ray absorber (UV-1)                                                                                                                                                       | 0.47 |
| Color-mixing preventive (Cpd-5)                                                                                                                                                       | 0.05 |
| Solvent (Solv-5)                                                                                                                                                                      | 0.24 |
| <u>5th Layer: Red-sensitive Layer</u>                                                                                                                                                 |      |
| Silver chlorobromide emulsion                                                                                                                                                         | 0.21 |

The compounds used were as follows.

## (ExY) Yellow coupler



## (ExM) Magenta coupler



## (ExC) Cyan coupler

A 1:3:6 mixture (by weight) of following compounds, wherein (R = H):(R = C<sub>2</sub>H<sub>5</sub>):(R = C<sub>4</sub>H<sub>9</sub>)



## (Cpd-1) Color image stabilizer



## (Cpd-3) Color image stabilizer



## (Cpd-4) Color image stabilizer



## (Cpd-5) Color mixing preventive agent

-continued



**(Cpd-6)** Color image stabilizer  
2:4:4 mixture (by weight) of (G):(H):(J)



**(Cpd-7)** Color image stabilizer



Average molecular weight 60,000

**(Cpd-8)** Color image stabilizer



**(Cpd-9)** Color image stabilizer



**(UV-I)** Ultraviolet absorbent

4:2:4 mixture (by weight) of (K):(L):(M)



-continued



and



(Solv-1) Solvent



(Solv-2) Solvent

1:1 (volume ratio) mixture of



(Solv-3) Solvent



(Solv-4) Solvent



(Solv-5) Solvent



(Solv-6) Solvent



The sample material prepared in the manner indicated above was designated as G.

After image exposure of this sample material G, continuous processing (a running test) was conducted until up to 2 times the development tank volume had been replenished, using an automatic development machine for paper and the processing stages and processing compositions noted below.

The composition of the color development solution was varied in the manner indicated in Table 4.

| Processing Stage  | Temperature | Time   | Replenishment quantity | Tank Capacity |
|-------------------|-------------|--------|------------------------|---------------|
| Color development | 38° C.      | 45 sec | 109 ml                 | 4 l           |
| Bleach-fixing     | 30-36° C.   | 45 sec | 215 ml                 | 4 l           |
| Stabilization (1) | 30-37° C.   | 20 sec | —                      | 2 l           |
| Stabilization (2) | 30-37° C.   | 20 sec | —                      | 2 l           |
| Stabilization (3) | 30-37° C.   | 20 sec | 364 ml                 | 2 l           |
| Drying            | 70-85° C.   | 60 sec | —                      | —             |

\*The replenishment quantity per 1 m<sup>2</sup> of photosensitive material

(A 3-tank counterflow system going from stabilization tank (1) to (3) was used.)

The compositions of the various processing solutions were as follows.

|                                                                                               | Tank<br>Solution | Replenisher<br>Solution |
|-----------------------------------------------------------------------------------------------|------------------|-------------------------|
| <b>Color Development Solution</b>                                                             |                  |                         |
| Water                                                                                         | 800 ml           | 800 ml                  |
| Ethylenediaminetetraacetic acid                                                               | 5.0 g            | 5.0 g                   |
| 5,6-Dihydroxybenzene-1,2,4-trisulfonic acid                                                   | 0.3 g            | 0.3 g                   |
| Triethanolamine                                                                               | 8.0 g            | 8.0 g                   |
| Sodium chloride                                                                               | See Table 4      | See Table 4             |
| Potassium bromide                                                                             |                  |                         |
| Potassium carbonate                                                                           | 25 g             | 25 g                    |
| Organic preservative A<br>(See Table 4)                                                       | 0.03 mol         | 0.05 mol                |
| N-ethyl-N-( $\beta$ -methanesulfonamidoethyl)-3-methyl-4-amino aniline sulfate                |                  |                         |
| Sulfuric acid salt                                                                            | 5.0 g            | 9.5 g                   |
| Sodium sulfite                                                                                | 0.1 g            | 0.2 g                   |
| Brightening agent<br>(Diaminostilbene agent<br>'WHITEX-4' manufactured by<br>Sumitomo Kagaku) | 1.0 g            | 2.5 g                   |
| Water added                                                                                   | 1000 ml          | 1000 ml                 |
| pH (25° C.)                                                                                   | 10.05            | 10.60                   |
| <b>Bleach-fix Solution (Same for both tank solution and replenisher solution)</b>             |                  |                         |
| Water                                                                                         | 400 ml           |                         |
| Ammonium thiosulfate (70%)                                                                    | 100 ml           |                         |
| Sodium sulfite                                                                                | 17 g             |                         |
| Ferric (III) ammonium ethylenediaminetetraacetate                                             | 55 g             |                         |
| Disodium ethylenediaminetetraacetate                                                          | 5 g              |                         |
| Glacial acetic acid                                                                           | 9 g              |                         |
| Water added                                                                                   | 1000 ml          |                         |
| pH (25° C.)                                                                                   | 5.40             |                         |
| <b>Stabilization Solution (Same for both tank solution and make-up solution)</b>              |                  |                         |
| Formalin (37%)                                                                                | 0.1 g            |                         |
| Formalin - sulfite adduct                                                                     | 0.7 g            |                         |
| 5-Chloro-2-methyl-4-isothiazolin-3-one                                                        | 0.02 g           |                         |
| 2-Methyl-4-isothiazolin-3-one                                                                 | 0.01 g           |                         |
| Copper sulfate                                                                                | 0.005 g          |                         |
| Aqueous ammonia (28%)                                                                         | 2.0 ml           |                         |
| Water added                                                                                   | 1000 ml          |                         |

-continued

|    | pH (25° C.)                                                                                                                                                                                                                                                                                                                                                                                                                                                                                  | 4.0                                                                                 |
|----|----------------------------------------------------------------------------------------------------------------------------------------------------------------------------------------------------------------------------------------------------------------------------------------------------------------------------------------------------------------------------------------------------------------------------------------------------------------------------------------------|-------------------------------------------------------------------------------------|
| 5  | The chloride ion concentration and bromide ion concentration in the replenishment solution were set such that the tank solution concentrations were maintained from the start to the end of the running processing.                                                                                                                                                                                                                                                                          |                                                                                     |
| 10 | The above sample coating material was subjected to graduated exposure for sensitometry using a sensitometer (FWH model manufactured by Fuji Photo Film Co., Ltd., light source color temperature 3200° K.). This was effected at exposures of 250 CMS for 1/10 second.                                                                                                                                                                                                                       |                                                                                     |
| 15 | Sensitometry as above was performed at the start and at the end of the running tests and a Macbeth densitometer was used to determine the blue (B) minimum density (D <sub>min</sub> ) and maximum density (D <sub>max</sub> ) on performance of the running test and the amount of change in the blue (B) minimum density that accompanied continuous processing (value at the end of the running test minus the value at the start of the running test). The results are noted in Table 4. |                                                                                     |
| 20 | The photosensitive material was also subjected to exposure to uniform light such as to make 90% of the coated silver developed silver and then, at the end of the running test, it was processed and the amount of developed silver and the amount of residual silver were determined by X ray fluorometry. The results are given in Table 4.                                                                                                                                                |                                                                                     |
| 25 | Further, at the end of the running test, the sample coating material was subjected to assessment of sensitization streaks in the same way as in Example 1. The assessment standards were in 4 stages as follows.                                                                                                                                                                                                                                                                             |                                                                                     |
| 30 |                                                                                                                                                                                                                                                                                                                                                                                                                                                                                              |                                                                                     |
| 35 |                                                                                                                                                                                                                                                                                                                                                                                                                                                                                              |                                                                                     |
|    | Sensitization<br>Streak Assessment                                                                                                                                                                                                                                                                                                                                                                                                                                                           | Number of Sensitization Streaks in<br>100 cm <sup>2</sup> (10 cm × 10 cm) of Sample |
|    | ○                                                                                                                                                                                                                                                                                                                                                                                                                                                                                            | 0                                                                                   |
|    | Δ                                                                                                                                                                                                                                                                                                                                                                                                                                                                                            | 1-2                                                                                 |
|    | ×                                                                                                                                                                                                                                                                                                                                                                                                                                                                                            | 3-5                                                                                 |
| 40 | xx                                                                                                                                                                                                                                                                                                                                                                                                                                                                                           | 6 or more                                                                           |

The results are given in Table 4.

TABLE 4

|                                                             | Development<br>Solution   | Processing I Example |                      |                      |                      |                      |                      |
|-------------------------------------------------------------|---------------------------|----------------------|----------------------|----------------------|----------------------|----------------------|----------------------|
|                                                             |                           | 1                    | 2                    | 3                    | 4                    | 5                    | 6                    |
| Chloride Ion<br>Concentration<br>(mol/l)                    | Tank<br>Solution          | $4.6 \times 10^{-2}$ | $1.0 \times 10^{-1}$ | $1.5 \times 10^{-1}$ | $4.6 \times 10^{-2}$ | $4.6 \times 10^{-2}$ | $4.6 \times 10^{-2}$ |
| Bromide Ion<br>Concentration<br>(mol/l)                     | Tank<br>Solution          | $1.3 \times 10^{-4}$ | $5.0 \times 10^{-4}$ | $1.0 \times 10^{-3}$ | $1.3 \times 10^{-4}$ | $5.0 \times 10^{-4}$ | $1.3 \times 10^{-4}$ |
| Organic<br>preservative A<br>Remarks                        | Replenishment<br>Solution | —                    | $5.5 \times 10^{-2}$ | $1.0 \times 10^{-1}$ | —                    | —                    | —                    |
| At start of<br>running test                                 | BL D <sub>max</sub>       | 2.38                 | 2.38                 | 2.37                 | 2.43                 | 2.42                 | 2.30                 |
| BL D <sub>min</sub>                                         | BL D <sub>min</sub>       | 0.08                 | 0.08                 | 0.08                 | 0.08                 | 0.08                 | 0.09                 |
| BL ΔD <sub>min</sub> (Value at<br>end minus value at start) |                           | +0.01                | ±0.00                | ±0.00                | ±0.00                | ±0.00                | +0.02                |
| Residual silver (μg/cm <sup>2</sup> )                       |                           | 1.3                  | 1.4                  | 1.6                  | 1.2                  | 1.4                  | 2.8                  |
| Sensitization<br>Streaks                                    |                           | ○                    | ○                    | ○                    | ○                    | ○                    | Δ                    |
| Processing I Example                                        |                           |                      |                      |                      |                      |                      |                      |
| Development<br>Solution                                     | Tank<br>Solution          | $5.0 \times 10^{-1}$ | $5.4 \times 10^{-2}$ | $5.0 \times 10^{-1}$ | $5.0 \times 10^{-1}$ | $5.4 \times 10^{-2}$ | $5.0 \times 10^{-1}$ |

TABLE 4-continued

| Chloride Ion Concentration (mol/l)                       | Replenishment Solution | $4.5 \times 10^{-1}$ | $0.8 \times 10^{-2}$ | $4.5 \times 10^{-1}$ | $4.5 \times 10^{-1}$                       | $0.8 \times 10^{-2}$                       | $4.9 \times 10^{-1}$                       |
|----------------------------------------------------------|------------------------|----------------------|----------------------|----------------------|--------------------------------------------|--------------------------------------------|--------------------------------------------|
| Development Solution                                     | Tank Solution          | $1.7 \times 10^{-4}$ | $5.9 \times 10^{-3}$ | $5.9 \times 10^{-3}$ | $1.7 \times 10^{-4}$                       | $5.9 \times 10^{-3}$                       | $5.9 \times 10^{-3}$                       |
| Bromide Ion Concentration (mol/l)                        | Replenishment Solution | $0.4 \times 10^{-4}$ | $5.8 \times 10^{-3}$ | $5.8 \times 10^{-3}$ | $0.4 \times 10^{-4}$                       | $5.8 \times 10^{-3}$                       | $5.8 \times 10^{-3}$                       |
| Organic preservative A Remarks                           |                        | I-1<br>Comparison    | I-1<br>Comparison    | I-1<br>Comparison    | Hydroxyl<br>amine<br>Comparison<br>Example | Hydroxyl<br>amine<br>Comparison<br>Example | Hydroxyl<br>amine<br>Comparison<br>Example |
| At start of running test                                 | BL D <sub>max</sub>    | 2.09                 | 1.89                 | 1.71                 | 1.98                                       | 1.76                                       | 1.66                                       |
| BL D <sub>in</sub>                                       |                        | 0.08                 | 0.08                 | 0.08                 | 0.09                                       | 0.09                                       | 0.08                                       |
| BL ΔD <sub>min</sub> (Value at end minus value at start) |                        | +0.01                | ±0.00                | ±0.00                | +0.02                                      | +0.02                                      | +0.01                                      |
| Residual silver (μg/cm <sup>2</sup> )                    |                        | 6.6                  | 9.9                  | 10.8                 | 7.2                                        | 11.1                                       | 12.6                                       |
| Sensitization Streaks                                    |                        | ○                    | ○                    | ○                    | Δ                                          | Δ                                          | Δ                                          |

It is apparent from Table 4 that in processing examples 1 to 6 in which processing was effected with development solutions of the invention, there were excellent photographic characteristics, since the maximum density was high and the minimum density was low, and that continuous processing was accompanied by hardly any increase in the minimum density.

The results were also good since the amount of residual silver was small and there were good sensitization streak prevention effects.

Use of the organic preservatives I-1 and II-19 gave still more desirable results, since in addition to the maximum density being higher and continuous processing being accompanied by little change in the minimum density, there was a reduction of residual silver and there were good pressure sensitization streak prevention effects.

As seen in processing example 6 to 12, when the chlorine ion concentration and bromine ion concentration were higher than the concentrations of the invention, the minimum density was low and pressure sensitization streaks were prevented by the maximum density was low and there was a large amount of residual silver, so such conditions were unsuitable for rapid processing.

#### EXAMPLE 6

The same procedure was used as in Example 5 except that in processing example 4, I-2, I-3, II-1, II-5, II-9, II-13 and II-20 were used instead of organic preservative A II-19. Similarly good results were obtained.

#### EXAMPLE 7

The same procedure as in Example 2 was followed except that in processing example 5, III-3, III-11, IV-1

and IV-2 were used instead of triethanolamine in the development solution similarly gave good results.

#### EXAMPLE 8

A multilayer color printing paper with the layer structure described below was prepared on a paper support laminated on both sides with polyethylene. The coating solutions were prepared as follows.

##### Preparation of 1st Layer Coating Solution

19.1 g of a yellow coupler (E×Y), 4.4 g of a color image stabilizer (Cpd-1) and 0.7 g of another color image stabilizer (Cpd-7) were dissolved by addition of 27.2 cc of ethyl acetate and 8.2 g of a solvent (Solv-3). This solution was emulsified and dispersed in 185 cc of a 10% gelatin aqueous solution containing 8 cc of 10% sodium dodecylbenzenesulfonate. Meanwhile, an emulsion was produced by adding to a silver chlorobromide emulsion (average cubic grain size 0.88 μm, cubic grains with a grain size distribution variation coefficient of 0.08 and having locally present 0.2 mol % silver bromide in some parts on grain surfaces) the two types of blue-sensitization dyes described below, in an amount that was  $2.0 \times 10^{-4}$  moles per 1 mole of silver in each case, and effecting sulfur sensitization. This emulsion and the emulsified dispersion described above were mixed and dissolved to give a 1st coating solution with the composition noted below. The coating solutions of the 2nd to 7th layers were prepared in the same manner. 1-Oxy-3,5-dichloro-s-triazine sodium salt was used as a gelatin hardener for each layer.

The following substances were used as spectral sensitization dyes in the various layers.

Blue-sensitive emulsion layer



-continued



$(2.0 \times 10^{-4}$  moles of each of the above 2 types per 1 mole of silver halide)

Green-sensitive emulsion layer



$(4.0 \times 10^{-4}$  moles per 1 mole of silver halide)

and



$(7.0 \times 10^{-5}$  moles per 1 mole of silver halide)

Red-sensitive emulsion layer



$(0.9 \times 10^{-4}$  moles per 1 mole of silver halide)

The following compound was added to the red-sensitive emulsion layer in an amount that was  $2.6 \times 10^{-3}$  moles per 1 mole of silver halide)

Also, to the blue-sensitive emulsion layer, green-sensitive emulsion layer and red-sensitive emulsion layer were added 1-(5-methylureidophenyl)-5-mercaptopotetrazole in amounts that were respectively  $8.5 \times 10^{-5}$  moles,  $7.7 \times 10^{-4}$  moles and  $2.5 \times 10^{-5}$  moles per 1 mole of silver halide.

The following dyes were added to the emulsion layers to prevent irradiation.



-continued

and



## Layer Structure

The compositions of the various layers were as follows. The figures indicate coating quantities (g/m<sup>2</sup>). Coating quantities calculated as silver are given for silver halide emulsions.

## Support

25

## Polyethylene-laminated paper.

(The polyethylene on the 1st layer side contains a white pigment (TiO<sub>2</sub>) and a blue dye (ultramarine).)

30

## 1st Layer: Blue-sensitive Layer

|                                               |      |
|-----------------------------------------------|------|
| Silver chlorobromide emulsion described above | 0.30 |
| Gelatin                                       | 1.86 |
| Yellow coupler (ExY)                          | 0.82 |
| Color image stabilizer (Cpd-1)                | 0.19 |
| Solvent (Solv-3)                              | 0.35 |
| Color image stabilizer (Cpd-7)                | 0.06 |

## 2nd Layer: Color-mixing Prevention Layer

|                                 |      |
|---------------------------------|------|
| Gelatin                         | 0.99 |
| Color-mixing preventive (Cpd-5) | 0.08 |
| Solvent (Solv-1)                | 0.16 |
| Solvent (Solv-4)                | 0.08 |

## 3rd Layer: Green-sensitive Layer

|                                                                                                                                                                                                                                                            |      |
|------------------------------------------------------------------------------------------------------------------------------------------------------------------------------------------------------------------------------------------------------------|------|
| Silver chlorobromide emulsion (1:3 (Ag moles ratio) mixture of cubic grains with average grain size of 0.55μ and 0.39 μm, grain size distribution variation coefficients respectively 0.10 and 0.08; 0.8 mol % AgBr are present locally on grain surfaces) | 0.12 |
| Gelatin                                                                                                                                                                                                                                                    | 1.24 |

40

35

45

50

## -continued

|                                                                                                                                                                                                                                                            |      |
|------------------------------------------------------------------------------------------------------------------------------------------------------------------------------------------------------------------------------------------------------------|------|
| Magenta coupler (ExM)                                                                                                                                                                                                                                      | 0.27 |
| Color image stabilizer (Cpd-3)                                                                                                                                                                                                                             | 0.15 |
| Color image stabilizer (Cpd-8)                                                                                                                                                                                                                             | 0.02 |
| Color image stabilizer (Cpd-9)                                                                                                                                                                                                                             | 0.03 |
| Solvent (Solv-2)                                                                                                                                                                                                                                           | 0.54 |
| <u>4th Layer: Ultraviolet Absorption Layer</u>                                                                                                                                                                                                             |      |
| Gelatin                                                                                                                                                                                                                                                    | 1.58 |
| Ultraviolet ray absorber (UV-1)                                                                                                                                                                                                                            | 0.47 |
| Color-mixing preventive (Cpd-5)                                                                                                                                                                                                                            | 0.05 |
| Solvent (Solv-5)                                                                                                                                                                                                                                           | 0.24 |
| <u>5th Layer: Red-sensitive Layer</u>                                                                                                                                                                                                                      |      |
| Silver chlorobromide emulsion (1:4 (Ag moles ratio) mixture of cubic grains with average grain size of 0.58μ and 0.45 μm, grain size distribution variation coefficients respectively 0.09 and 0.11; 0.6 mol % AgBr are present locally on grain surfaces) | 0.23 |
| Gelatin                                                                                                                                                                                                                                                    | 1.34 |
| Cyan coupler (ExC)                                                                                                                                                                                                                                         | 0.32 |
| Color image stabilizer (Cpd-6)                                                                                                                                                                                                                             | 0.17 |
| Color image stabilizer (Cpd-10)                                                                                                                                                                                                                            | 0.04 |
| Color image stabilizer (Cpd-7)                                                                                                                                                                                                                             | 0.40 |
| Solvent (Solv-6)                                                                                                                                                                                                                                           | 0.15 |
| <u>6th Layer: Ultraviolet Absorption Layer</u>                                                                                                                                                                                                             |      |
| Gelatin                                                                                                                                                                                                                                                    | 0.53 |
| Ultraviolet ray absorber (UV-1)                                                                                                                                                                                                                            | 0.16 |
| Color-mixing preventive (Cpd-5)                                                                                                                                                                                                                            | 0.02 |
| Solvent (Solv-5)                                                                                                                                                                                                                                           | 0.08 |
| <u>7th Layer: Protective Layer</u>                                                                                                                                                                                                                         |      |
| Gelatin                                                                                                                                                                                                                                                    | 1.33 |
| Acryl-modified polyvinyl alcohol copolymer (modification degree 17%)                                                                                                                                                                                       | 0.17 |
| Liquid paraffin                                                                                                                                                                                                                                            | 0.03 |

50 The compounds used were as follows.

## (ExY) Yellow coupler



## (ExM) Magenta coupler

-continued



(ExC) Cyan coupler  
A 2:4:4 mixture (by weight) of (Compound (N)  
wherein R = C<sub>2</sub>H<sub>5</sub>):(Compound (N) wherein R = C<sub>4</sub>H<sub>9</sub>):(O)



### (Cpd-1) Color image stabilizer



**(Cpd-3) Color image stabilizer**



**(Cpd-5) Color mixing preventive**



**(Cpd-6) Color image stabilizer**  
2:4:4 mixture (by weight) of (P):(Q):(R)

59

5,066,571

60

-continued



### (Cpd-7) Color image stabilizer



### (Cpd-8) Color image stabilizer



**(Cpd-9) Color image stabilizer**



**(Cpd-10) Color image stabilizer**



**(UV-1) Ultraviolet absorbent**  
4:2:4 mixture (by weight) of (S):(T):(U)



-continued



### (Solv-1) Solvent



(Solv-2) Solvent  
2:1 (by volume) mixture of



(Solv-3) Solvent  
 $O=P(O-C_9H_{19(iso)})_3$

### (Solv-4) Solvent



(Solv-5) Solvent  
 $\text{COOC}_8\text{H}_{17}$

$$\begin{array}{c} \cdot \\ | \\ (\text{CH}_2)_8 \\ | \\ \text{COOC}_8\text{H}_{17} \end{array}$$

### (Solv-6) Solvent



The sample material thus prepared was designated as H.

Next, samples H to L were prepared by following the same procedure as for H but varying the amounts of coated silver in the various emulsion layers to the values noted in Table 5.

TABLE 5

| Coating Sample | Coated Silver Quantity (g/m <sup>2</sup> ) |      |      |       |
|----------------|--------------------------------------------|------|------|-------|
|                | B                                          | G    | R    | Total |
| H              | 0.30                                       | 0.12 | 0.23 | 0.65  |
| I              | 0.32                                       | 0.18 | 0.25 | 0.75  |
| J              | 0.34                                       | 0.19 | 0.27 | 0.80  |
| K              | 0.37                                       | 0.22 | 0.31 | 0.90  |

TABLE 5-continued

| Coating Sample | Coated Silver Quantity (g/m <sup>2</sup> ) |      |      |       |
|----------------|--------------------------------------------|------|------|-------|
|                | B                                          | G    | R    | Total |
| L              | 0.40                                       | 0.25 | 0.35 | 1.00  |

65 After image exposure of samples H to L, continuous processing (a running test) was conducted until up to 2 times the development tank's volume had been replenished, using an automatic development machine for paper and the processing stages and processing compositions noted below.

| Processing Stage  | Temp-erature | Time   | Replenish-ment quantity | Tank Capacity |
|-------------------|--------------|--------|-------------------------|---------------|
| Color development | 38° C.       | 45 sec | See Table 6             | 4 l           |
| Bleach-fixing     | 30-36° C.    | 45 sec | 61 ml                   | 4 l           |
| Washing (1)       | 30-37° C.    | 30 sec | —                       | 2 l           |
| Washing (2)       | 30-37° C.    | 30 sec | —                       | 2 l           |
| Washing (3)       | 30-37° C.    | 30 sec | 364 ml                  | 2 l           |
| Drying            | 70-85° C.    | 60 sec |                         |               |

\*The replenishment quantity per 1 m<sup>2</sup> of photosensitive material

(A 3-tank counterflow system running from washing tank (1) to (3) was used. The bleach-fix bath was replenished with 122 ml of washing (1) solution per 1 m<sup>2</sup> of photosensitive material.)

The compositions of the various processing solutions were as follows.

Color Development Solution (Tank Solution)

|                                                                                                  |             |
|--------------------------------------------------------------------------------------------------|-------------|
| Water                                                                                            | 800 ml      |
| Ethylenediamine-N,N,N',N'-tetramethylenephosphonic acid                                          | 3.0 g       |
| Triethanolamine                                                                                  | 8.0 g       |
| Sodium chloride                                                                                  | See Table 6 |
| Potassium bromide                                                                                | See Table 6 |
| Potassium carbonate                                                                              | 25 g        |
| N-ethyl-N-( $\beta$ -methanesulfonamidoethyl)-3-methyl-4-aminoaniline sulfate sulfuric acid salt | 5.0 g       |
| Organic preservative A (II-19)                                                                   | 0.03 mol    |
| Brightening agent (WHITEX-4 manufactured by Sumitomo Kagaku)                                     | 1.0 g       |
| Water added                                                                                      | 1000 ml     |
| pH (25° C.)                                                                                      | 10.05       |

|   |                                                                                        |
|---|----------------------------------------------------------------------------------------|
| 5 | tank solution.<br>Washing Water (Same for both tank solution and replenisher solution) |
|   | Ion exchange purified water (both calcium and magnesium at 3 ppm or less)              |

During continuous processing, corrections of concentration due to evaporation were made by adding to the color development solution, bleach-fix solution and washing solution additions of distilled water corresponding to the amounts of evaporated water.

The above sample coating material was subjected to graduated exposure for sensitometry using a sensitometer (FWH model manufactured by Fuji Photo Film Co., Ltd., light source color temperature 3200° K.). This was effected at exposures of 250 CMS for 1/10 second.

Sensitometry as above was performed at the start and at the end of the running tests and a Macbeth densitometer was used to determine the blue (B) minimum density (D<sub>min</sub>) and maximum density (D<sub>max</sub>) on performance of the running test and the amount of change in the blue (B) minimum density that accompanied continuous processing (value at the end of the running test minus value at the start of the running test). The results are described in Table 6.

The photosensitive material was also subjected to exposure to uniform light such sufficient to make 90% of the coated silver developed silver and then, at the end of the running test, it was processed and the amount of developed silver and the amount of residual silver were determined by X ray fluorometry. Findings are given in Table 6.

|                                                                                                  | Replenishment Solution (a) | Replenishment Solution (b) | Replenishment Solution (c) | Replenishment Solution (d) |
|--------------------------------------------------------------------------------------------------|----------------------------|----------------------------|----------------------------|----------------------------|
| <u>Developer Replenishment Solution</u>                                                          |                            |                            |                            |                            |
| Ethylenediamine-N,N,N',N'-tetra-methylenephosphonic acid                                         | 3 (g/l)                    | 3 (g/l)                    | 3 (g/l)                    | 5 (g/l)                    |
| Triethanolamine                                                                                  | 12 (g/l)                   | 12 (g/l)                   | 12 (g/l)                   | 12 (g/l)                   |
| Potassium chloride                                                                               | See table 6                | See Table 6                | See table 6                | See Table 6                |
| Potassium bromide                                                                                | See table 6                | See Table 6                | See table 6                | See Table 6                |
| Potassium carbonate                                                                              | 26 (g/l)                   | 26 (g/l)                   | 26 (g/l)                   | 26 (g/l)                   |
| N-Ethyl-N-( $\beta$ -methanesulfonamidoethyl)-3-methyl-4-aminoaniline sulfate sulfuric acid salt | 6 (g/l)                    | 7 (g/l)                    | 9 (g/l)                    | 15 (g/l)                   |
| Organic preservative (II-19)                                                                     | 6 (g/l)                    | 6 (g/l)                    | 7 (g/l)                    | 9 (g/l)                    |
| Brightening agent (WHITEX-4 manufactured by Sumitomo Kagaku)                                     | 1.5 (g/l)                  | 2 (g/l)                    | 2.5 (g/l)                  | 3 (g/l)                    |
| pH (25° C.) (adjusted with KOH or H <sub>2</sub> SO <sub>4</sub> )                               | 10.35                      | 10.45                      | 10.55                      | 11.00                      |

Bleach-fix Solution

|                                                    |         |
|----------------------------------------------------|---------|
| Water                                              | 400 ml  |
| Ammonium thiosulfate (70%)                         | 100 ml  |
| Ammonium sulfite                                   | 38 g    |
| Ferric (III) ammonium ethylene-diaminetetraacetate | 55 g    |
| Disodium ethylenediaminetetraacetate               | 5 g     |
| Glacial acetic acid                                | 9 g     |
| Water added                                        | 1000 ml |
| pH (25° C.)                                        | 5.40    |
| (Replenishment solution)                           |         |

The solution was concentrated in 2.5 times of the

Further, at the end of the running test, the sample coating material was subjected to assessment of sensitization streaks in the same way as in Example 1. The assessment standards were in 4 stages as follows.

|    | Sensitization Streak Assessment | Number of Sensitization Streaks in 100 cm <sup>2</sup> (10 cm × 10 cm) of Sample |
|----|---------------------------------|----------------------------------------------------------------------------------|
| 60 | ○                               | 0                                                                                |
|    | Δ                               | 1-2                                                                              |
|    | X                               | 3-5                                                                              |
|    | XX                              | 6 or more                                                                        |

65 The assessment findings are given in Table 4.

TABLE 6

Processing I Example

TABLE 6-continued

|                                                                          |                        | 1                    | 2                    | 3                    | 4                    | 5                    | 6                    | 7                    |
|--------------------------------------------------------------------------|------------------------|----------------------|----------------------|----------------------|----------------------|----------------------|----------------------|----------------------|
| Coating Sample                                                           |                        | H                    | H                    | H                    | H                    | H                    | H                    | H                    |
| Replenishment Solution                                                   |                        | (c)                  | (c)                  | (c)                  | (c)                  | (a)                  | (b)                  | (c)                  |
| Replenishment quantity (per 1 m <sup>2</sup> of photosensitive material) |                        | 100 ml               | 100 ml               | 100 ml               | 100 ml               | 300 ml               | 200 ml               | 100 ml               |
| Development Solution                                                     | Tank Solution          | $4.3 \times 10^{-2}$ | $5.0 \times 10^{-1}$ | $1.0 \times 10^{-1}$ | $1.5 \times 10^{-1}$ | $3.6 \times 10^{-2}$ | $6 \times 10^{-2}$   | $6 \times 10^{-2}$   |
| Chloride Ion Concentration (mol/l)                                       | Replenishment Solution | —                    | $0.7 \times 10^{-2}$ | $5.7 \times 10^{-2}$ | $1.0 \times 10^{-2}$ | $2.2 \times 10^{-2}$ | $4 \times 10^{-2}$   | $1.7 \times 10^{-2}$ |
| Development Solution                                                     | Tank Solution          | $1.2 \times 10^{-4}$ | $5.0 \times 10^{-4}$ | $1.0 \times 10^{-3}$ | $1.0 \times 10^{-3}$ | $4.0 \times 10^{-5}$ | $2 \times 10^{-4}$   | $2 \times 10^{-4}$   |
| Bromide Ion Concentration (mol/l)                                        | Replenishment Solution | —                    | $3.8 \times 10^{-4}$ | $9.0 \times 10^{-4}$ | $9.0 \times 10^{-4}$ | $2.0 \times 10^{-5}$ | $1.4 \times 10^{-4}$ | $8 \times 10^{-5}$   |
| Remarks                                                                  |                        | Invention            | Invention            | Invention            | Invention            | Invention            | Invention            | Invention            |
| At start                                                                 | BL D <sub>max</sub>    | 2.30                 | 2.30                 | 2.24                 | 2.20                 | 2.31                 | 2.30                 | 2.30                 |
|                                                                          | BL D <sub>min</sub>    | 0.07                 | 0.07                 | 0.07                 | 0.07                 | 0.08                 | 0.07                 | 0.07                 |
| BL ΔD <sub>min</sub> (Value at end minus value at start)                 |                        | +0.01                | ±0.00                | ±0.00                | ±0.00                | +0.02                | ±0.00                | ±0.00                |
| Residual silver (μg/m <sup>2</sup> )                                     |                        | 1.0                  | 1.0                  | 1.9                  | 2.4                  | 2.5                  | 1.0                  | 1.0                  |
| Sensitization Streaks                                                    |                        | ○                    | ○                    | ○                    | ○                    | ○                    | ○                    | ○                    |
| Processing I Example                                                     |                        |                      |                      |                      |                      |                      |                      |                      |
|                                                                          |                        | 8                    | 9                    | 10                   | 11                   | 12                   | 13                   | 14                   |
| Coating Sample                                                           |                        | H                    | H                    | I                    | J                    | K                    | L                    | H                    |
| Replenishment Solution                                                   |                        | (d)                  | (c)                  | (c)                  | (c)                  | (c)                  | (c)                  | (a)                  |
| Replenishment quantity (per 1 m <sup>2</sup> of photosensitive material) |                        | 30 ml                | 100 ml               | 100 ml               | 100 ml               | 100 ml               | 100 ml               | 300 ml               |
| Development Solution                                                     | Tank Solution          | $1.2 \times 10^{-1}$ | $7 \times 10^{-2}$   | $7 \times 10^{-2}$   | $7 \times 10^{-2}$   | $7 \times 10^{-2}$   | $7 \times 10^{-2}$   | $1.4 \times 10^{-2}$ |
| Chloride Ion Concentration (mol/l)                                       | Replenishment Solution | —                    | $2.7 \times 10^{-2}$ | $2.5 \times 10^{-2}$ | $2.2 \times 10^{-2}$ | $2.0 \times 10^{-2}$ | $1.7 \times 10^{-2}$ | —                    |
| Development Solution                                                     | Tank Solution          | $7 \times 10^{-4}$   | $2.5 \times 10^{-4}$ | $2.5 \times 10^{-4}$ | $2.5 \times 10^{-4}$ | $2.5 \times 10^{-4}$ | $2.5 \times 10^{-4}$ | $2.0 \times 10^{-5}$ |
| Bromide Ion Concentration (mol/l)                                        | Replenishment Solution | $3.5 \times 10^{-4}$ | $1.3 \times 10^{-4}$ | $1.0 \times 10^{-4}$ | $0.6 \times 10^{-4}$ | $0.3 \times 10^{-4}$ | —                    | —                    |
| Remarks                                                                  |                        | Invention            | Invention            | Invention            | Invention            | Invention            | Invention            | Comparison Example   |
| At start                                                                 | BL D <sub>max</sub>    | 2.21                 | 2.30                 | 2.31                 | 2.30                 | 2.25                 | 2.20                 | 2.30                 |
|                                                                          | BL D <sub>min</sub>    | 0.07                 | 0.07                 | 0.07                 | 0.07                 | 0.08                 | 0.08                 | 0.09                 |
| BL ΔD <sub>min</sub> (Value at end minus value at start)                 |                        | +0.02                | ±0.00                | ±0.00                | +0.01                | +0.02                | +0.02                | +0.08                |
| Residual silver (μg/m <sup>2</sup> )                                     |                        | 2.3                  | 1.1                  | 1.3                  | 2.0                  | 3.3                  | 3.9                  | 9.8                  |
| Sensitization Streaks                                                    |                        | ○                    | ○                    | ○                    | Δ                    | Δ                    | Δ                    | XX                   |
| Processing I Example                                                     |                        |                      |                      |                      |                      |                      |                      |                      |
|                                                                          |                        | 15                   | 16                   | 17                   | 18                   | 19                   | 20                   |                      |
| Coating Sample                                                           |                        | H                    | I                    | I                    | I                    | H                    | H                    |                      |
| Replenishment Solution                                                   |                        | (d)                  | (a)                  | (b)                  | (d)                  | (a)                  | (a)                  |                      |
| Replenishment quantity (per 1 m <sup>2</sup> of photosensitive material) |                        | 30 ml                | 300 ml               | 200 ml               | 30 ml                | 300 ml               | 300 ml               |                      |
| Development Solution                                                     | Tank Solution          | $2.0 \times 10^{-1}$ | $5.4 \times 10^{-2}$ | $5.4 \times 10^{-2}$ | $2.0 \times 10^{-1}$ | $5.4 \times 10^{-2}$ | $5.4 \times 10^{-2}$ | $5.4 \times 10^{-2}$ |
| Chloride Ion Concentration (mol/l)                                       | Replenishment Solution | $6.0 \times 10^{-2}$ | $4.0 \times 10^{-2}$ | $3.3 \times 10^{-2}$ | $6.0 \times 10^{-2}$ | $4.0 \times 10^{-2}$ | $4.0 \times 10^{-2}$ | $4.0 \times 10^{-2}$ |
| Development Solution                                                     | Tank Solution          | $1.7 \times 10^{-3}$ | $1.7 \times 10^{-3}$ | $5.9 \times 10^{-3}$ | $3.6 \times 10^{-4}$ | $1.7 \times 10^{-3}$ | $5.9 \times 10^{-3}$ | $5.9 \times 10^{-3}$ |
| Bromide Ion Concentration (mol/l)                                        | Replenishment Solution | $1.5 \times 10^{-3}$ | $1.7 \times 10^{-3}$ | $5.9 \times 10^{-3}$ | —                    | $1.7 \times 10^{-3}$ | $5.9 \times 10^{-3}$ | $5.9 \times 10^{-3}$ |
| Remarks                                                                  |                        | Comparison Example   | Comparison Example   | Comparison Example   | Comparison Example   | Comparison Example   | Comparison Example   | Comparison Example   |
| At start                                                                 | BL D <sub>max</sub>    | 1.70                 | 1.84                 | 1.66                 | 1.90                 | 1.80                 | 1.62                 |                      |
|                                                                          | BL D <sub>min</sub>    | 0.07                 | 0.07                 | 0.07                 | 0.08                 | 0.07                 | 0.07                 | 0.07                 |
| BL ΔD <sub>min</sub> (Value at end minus value at start)                 |                        | +0.04                | +0.01                | +0.01                | +0.05                | +0.02                | +0.01                |                      |
| Residual silver (μg/m <sup>2</sup> )                                     |                        | 8.9                  | 10.0                 | 10.6                 | 6.9                  | 5.0                  | 8.1                  |                      |
| Sensitization Streaks                                                    |                        | Δ                    | Δ                    | ○                    | Δ                    | Δ                    | Δ                    |                      |

It is seen from Table 6 that in processing examples (1) to (13) in which processing was effected with development solutions of the invention gave good results, since the photographic characteristics were excellent; the

maximum density was high and the minimum density was low, and continuous processing was accompanied by hardly any increase in the minimum density.

With the examples of the invention, when the development solution's chlorine ion concentration was  $4 \times 10^{-2}$  to  $1 \times 10^{-1}$  mol/l and its bromine ion concentration was  $5 \times 10^{-5}$  to  $5 \times 10^{-4}$  mol/l, the results were better in respect of the maximum density, increase in the minimum density during running processing and the amount of residual silver, as seen in processing examples (1) to (8).

Again with the examples of the invention, when the photosensitive material's coated silver content was 0.8 g/m<sup>2</sup> or less as in processing examples (9) to (13) the results in respect of the maximum density, increase in the minimum density during running processing and the amount of residual silver and occurrence of sensitization streaks were still better, and they were even better when the amount of coated silver was 0.75 g/m<sup>2</sup> or less.

As seen in processing examples (14) to (20), when the chlorine ion concentration and bromine ion concentration were lower than the concentrations of the invention, although the maximum density was high there was a great increase in the minimum density during running processing and there was a great amount of residual silver and marked occurrence of sensitization streaks. In cases where either the chlorine ion or bromine ion concentration was higher than the concentration of the invention, a loss of maximum density and an increase in the amount of residual silver.

Making a direct comparison for the same photo sensitive material and replenishment quantity, the results in processing examples (5), (14), (19) and (20) clearly show that combinations of chlorine ion and bromine ion concentrations of the invention provided excellent results.

#### EXAMPLE 9

The same procedure as in Example 8 was followed, except that in processing example (1), I-1, I-2, I-3, II-2, II-1, II-5, II-9, II-13 and II-20 were used instead of organic preservative A II-19. Similarly good results were obtained.

#### EXAMPLE 10

The same procedure as in Example 8 was followed, except that in processing stage (1) III-3, III-11, IV-1 and IV-7 were used instead of triethanolamine in the development solution. Similarly good results were obtained.

While the invention has been described in detail and with reference to specific embodiments thereof, it will be apparent to one skilled in the art that various changes and modifications can be made therein without departing from the spirit and scope thereof.

What is claimed is:

1. A method for processing a silver halide color photosensitive material which comprises developing a color photographic light-sensitive material comprising a support having thereon having at least one light-sensitive silver halide emulsion layer containing a silver halide comprising at least 98 mol % silver chloride;

in a color developer solution comprising a primary amine color developing agent, and having a chloride concentration of from  $4 \times 10^{-2}$  to  $1 \times 10^{-1}$  mol/l, and a bromide ion concentration of from  $5.0 \times 10^{-5}$  to  $5 \times 10^{-4}$  mol/l.

2. The method as claimed in claim 1, wherein said developer solution comprises from 0.005 to 0.5 mol/l of an organic preservative represented by formulae (I) or (II):



(I)

5 wherein R<sup>11</sup> and R<sup>12</sup> each represents hydrogen, an unsubstituted or substituted alkyl group, an unsubstituted or substituted alkenyl group, an unsubstituted or substituted aryl group or a substituted or unsubstituted heteroaromatic group, provided that at least one of R<sup>11</sup> and R<sup>12</sup> is a group other than hydrogen, and R<sup>11</sup> and R<sup>12</sup> may be linked to form a saturated or unsaturated 5-membered or 6-membered heterocyclic ring; and



(II)

15 10 20 25 30 35 wherein R<sup>31</sup>, R<sup>32</sup> and R<sup>33</sup> each represents hydrogen, a substituted or unsubstituted alkyl group, a substituted or unsubstituted aryl group, or a substituted or unsubstituted heterocyclic group; R<sup>34</sup> represents a hydroxyl group, a hydroxyamino group, a substituted or unsubstituted alkyl group, a substituted or unsubstituted aryl group, a substituted or unsubstituted heterocyclic group, a substituted or unsubstituted alkoxy group, a substituted or unsubstituted aryloxy group, a substituted or unsubstituted carbamoyl group or a substituted or unsubstituted amino group; X<sup>31</sup> represents —CO—, —SO<sub>2</sub>— or —C(=NH)—; and n is 0 or 1; provided that when n is 0, R<sup>34</sup> represents an alkyl group, aryl group or heterocyclic group; and R<sup>33</sup> and R<sup>34</sup> may be linked to form a heterocyclic ring.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 952

8. The method as claimed in claim 1, wherein said color development step is performed at a temperature of 30° to 40° C. for a developing time of 30 seconds to 2 minutes.

9. The method as claimed in claim 8, wherein the total processing time from the first contact of said color light-sensitive material with said developer solution until said light-sensitive material is removed from a final bath is at most 4 minutes.

10. The method as claimed in claim 1, wherein said light-sensitive silver halide emulsion layer contains at most 0.80 g/m<sup>2</sup> of silver in said silver halide.

11. The method as claimed in claim 10, wherein said light-sensitive silver halide emulsion layer contains at most 0.75 g/m<sup>2</sup> of silver in said silver halide.

12. The method as claimed in claim 11, wherein said light-sensitive silver halide emulsion layer contains from 0.3 to 0.65 g/m<sup>2</sup> of silver in said silver halide.

13. The method as claimed in claim 1, wherein said color developer solution is substantially free from benzyl alcohol.

14. The method as claimed in claim 1, wherein said light-sensitive silver halide emulsion layer further comprises a pyrazoloazole coupler; at least one compound represented by formula (FI) or (FII); and at least one compound represented by formula (GI):



(FI)



(FII)

wherein R<sup>1</sup> and R<sup>2</sup> each represents an aliphatic group, an aromatic group or a heterocyclic group; n is 1 or 0; A represents a group capable of forming a chemical bond by reacting with a primary aromatic amine developing agent; X represents a group which is eliminated upon said reaction of A with said primary aromatic amine developing agent; B represents hydrogen, an aliphatic group, an aromatic group, a heterocyclic group, an acyl group or a sulfonyl group; and Y represents a group capable of accelerating the addition of said aromatic amine developing agent to said compound represented by formula (FII), provided that R<sub>1</sub> and X, Y and R<sub>2</sub> or Y and B may be linked to form a cyclic structure; and



(GI)

wherein R represents an aliphatic group, an aromatic group or a heterocyclic group; and Z represents a nucleophilic group or a group which is decomposed in said photosensitive material after development to release a nucleophilic group.

\* \* \* \* \*

30

35

40

45

50

55

60

65